

Aug. 17, 1965

F. C. HULL

3,201,233

CRACK RESISTANT STAINLESS STEEL ALLOYS

Filed June 13, 1962

6 Sheets-Sheet 1



Fig.1.



Fig.2.

WITNESSES:

Leon J. Vaga  
James T. Young

INVENTOR

Frederick C. Hull  
BY *H. M. Snyder*  
ATTORNEY

Aug. 17, 1965

F. C. HULL

3,201,233

CRACK RESISTANT STAINLESS STEEL ALLOYS

Filed June 13, 1962

6 Sheets-Sheet 2



Fig.3.



Fig.4.

Aug. 17, 1965

F. C. HULL

3,201,233

CRACK RESISTANT STAINLESS STEEL ALLOYS

Filed June 13, 1962

6 Sheets-Sheet 3



Fig. 5.



Fig. 9

Aug. 17, 1965

F. C. HULL

3,201,233

CRACK RESISTANT STAINLESS STEEL ALLOYS

Filed June 13, 1962

6 Sheets-Sheet 4



Fig. 6



Fig. 7

Aug. 17, 1965

F. C. HULL

3,201,233

CRACK RESISTANT STAINLESS STEEL ALLOYS

Filed June 13, 1962

6 Sheets-Sheet 5



Fig. 8



Fig. 12

Aug. 17, 1965

F. C. HULL

3,201,233

CRACK RESISTANT STAINLESS STEEL ALLOYS

Filed June 13, 1962

6 Sheets-Sheet 6



Fig. 10



Fig. 11



Fig. 13

## 1

3,201,233

**CRACK RESISTANT STAINLESS STEEL ALLOYS**  
Frederick C. Hull, Pittsburgh, Pa., assignor to Westinghouse Electric Corporation, East Pittsburgh, Pa., a corporation of Pennsylvania

Filed June 13, 1962, Ser. No. 202,220  
11 Claims. (Cl. 75—128)

This application is a continuation-in-part of application Serial No. 7,449, filed February 8, 1960, now abandoned.

This invention is directed to a family of novel high-manganese stainless steel alloys containing molybdenum and to articles made from these alloys; the alloys exhibiting greatly improved resistance to various types of hot-cracking in the as-cast and as-welded condition as well as other desirable properties.

Stainless steel alloys are commonly employed in the manufacture of articles and structures for use at elevated temperature or in corrosive environments. Thus, retorts, pumps, valves, and pressure vessels of various types are often cast in stainless steel. Wrought stainless steel articles such as steam chests, piping for boilers and turbines, and other conduits are also commonly subjected to operation in these difficult environments. In many of these devices welds must be made to unite casting to casting, wrought member to wrought member, and casting to wrought member.

It has been found that the solidification of stainless steels, and particularly of fully austenitic stainless steels, from the molten condition is often accompanied by the formation of cracks which tend to impair or destroy the usefulness of the article manufactured. When this phenomenon occurs in castings it is termed "hot-tearing," and when it occurs in weld metal it is termed "hot-cracking" or "microfissuring."

The hot-tearing phenomenon often occurs when an austenitic stainless steel casting of complex shape is poured into a mold which is too rigid to allow free contraction of the casting during cooling. Castings having long thin sections immediately adjacent to heavier sections are especially prone to cracking.

The problem of cracking of welds is particularly acute in the field of high temperature, high-stress applications where welds must be made to join heavy sections of stainless steel held under restraint. Steam turbines, boilers, and chemical processing equipment require welded sections of this description. The microfissuring of welds actually has two aspects. The first, which is the hot-cracking in the weld deposit which often occurs upon solidification of molten austenitic stainless steel, has been briefly mentioned above. The second aspect is a cracking phenomenon related to those described above, but which occurs in the heat-affected zone of either wrought or cast base metal during welding of heavy sections. The volume of base metal adjacent to the molten weld metal undergoes rapid heating to a temperature close to the melting point followed by cooling to ambient temperature. This rapid heating and cooling cycle, combined with the stresses imposed by hindered thermal contraction, has been found to severely damage the base metal of many stainless steels of the prior art. The damage is evidenced by cracking which originates in the grain boundaries of the base metal.

Stainless steels of the AISI types 304, 316, 321, and 347 were developed many years ago to resist general corrosion, pitting, and grain boundary attack. When it became evident that these austenitic stainless steels, and in par-

## 2

ticular AISI types 316, 321, and 347 had much higher creep strength than ferritic steels, they were applied in many high temperature, high-stress situations as the best available materials. The application of fully austenitic alloys such as the alloys of the AISI 300 series mentioned above, is limited by the susceptibility of certain of these alloys to hot-tearing when cast to shape as large components and to hot-cracking during the welding of restrained joints.

Since the apparatus used at elevated temperatures, such as steam chest, steam-turbine piping, and chemical retorts, has great importance for industry, the problems of hot-tearing and weld cracking have been the subject of intense investigation. These cracking phenomena appear to result from the lack of ability of the metal grains to hold together when subjected to tensile stresses at temperatures just below the solidus or perhaps in some cases while trace films of liquid are still present between some grains. The exact mechanism by which this high temperature cracking occurs is not understood, nor is there any known method for healing the cracks once they have formed. Wide variation has been found in the susceptibility to cracking even within a given grade of steel, and there is as yet, no satisfactory explanation for this variation. Uncertainty as to the quality of the welded joints has meant that excessive time and money are expended for testing, inspection, and repair welding to prevent service failures in critical applications such as have been mentioned above.

It is a primary object of this invention to provide novel stainless steel alloys having improved resistance to hot-tearing and hot-cracking and high creep rupture strength, and which are suitable for use as castings, as wrought products, and as welding rod, which include, in predetermined proportions, the elements iron, chromium, nickel, and manganese, with predetermined amounts of molybdenum.

It is a further object of this invention to provide a novel stainless steel alloy for use as castings, as wrought members, and as welding rod having improved resistance to hot-tearing and hot-cracking, which includes, in predetermined proportions, the elements iron, chromium, nickel, manganese and molybdenum, in which the total percent of manganese and molybdenum is a critical consideration.

A further object of this invention is to provide a substantially austenitic stainless steel alloy having good resistance to hot-cracking and hot-tearing, and improved strength and corrosion resistance, which includes in predetermined amounts the elements iron, chromium, nickel, manganese, molybdenum and at least one carbide stabilizer selected from the group consisting of titanium and columbium.

It is still another object of this invention to provide a welding electrode capable of depositing a stainless steel weld bead resistant to microfissuring as a joint between substantially austenitic stainless steel members and having an essentially austenitic structure which includes, in predetermined amounts, the elements iron, chromium, nickel, manganese, and molybdenum.

Yet another object of this invention is to provide a crack resistant substantially austenitic stainless steel having relatively high strength including, in predetermined proportions, the elements iron, chromium, nickel, manganese and molybdenum as a base alloy, with small but critical additions of vanadium, boron, zirconium and nitrogen.

Still another object of this invention is the provision of weldable austenitic stainless steels which are useful at sub-zero temperatures and specifically for cryogenic applications involving the handling of liquefied gases, such as liquid nitrogen, hydrogen or helium.

Other objects of the invention will, in part, be obvious, and will, in part, appear hereinafter.

The nature of the invention will be more readily understood from the following description taken in conjunction with the figures, in which:

FIGURE 1 is a typical CPT test (which is hereinafter defined) curve in which cracking index is plotted against arbitrary mold numbers;

FIG. 2 is a graph plotting CPT test mold numbers for a cracking index of 40 against weight percent of some common alloying additives in stainless steel;

FIG. 3 is a graph similar to FIG. 2 for certain other additives in stainless steel;

FIG. 4 is a hot-cracking curve for manganese in which CPT test mold numbers for cracking indices (CI) of 40 and zero are plotted against weight percent of manganese;

FIG. 5 is a graph in which percent molybdenum is plotted against percent manganese and contours are drawn to indicate compositions having equal cracking characteristics;

FIG. 6 is an illustration of a simplified impact test;

FIG. 7 is a graph in which bend angle is plotted against chromium content for alloys of this invention;

FIG. 8 is a graph in which bend angle is plotted against the composition function;

FIG. 9 is a graph showing the effects of nickel and manganese and delta ferrite on the cracking of stainless steels in which average cracking index in a No. 6 CPT test mold is plotted against percent nickel;

FIG. 10 is a graph in which stress rupture strength is plotted against nitrogen content for weldable stainless steels and for high strength weldable stainless steel;

FIG. 11 is a graph similar to FIG. 10 in which creep strength is plotted against nitrogen content for the same groups of steels;

FIG. 12 is a graph in which elongation at rupture is plotted against nitrogen content for alloys of this invention; and

FIG. 13 is a graph in which yield and tensile strengths of alloys at room temperature and 1025° F. are plotted against nitrogen content.

This invention is directed to a family of weldable stainless steel alloys containing iron, nickel, chromium and molybdenum which owe their distinctiveness in large degree to the uncommonly high proportion of manganese which they contain and the unique relationship between manganese and molybdenum. This alloy family includes member alloys having a wide range of characteristics which result from modifications of the basic composition either by changing the proportions thereof and/or adding other alloying elements. These alloys are fully or highly austenitic.

In the broadest sense the fully austenitic weldable alloys of this invention comprise, by weight, from 14% to 20% chromium, from 15% to 30% nickel, from 7.5% to 15% manganese, from 0.5% to 3.75% molybdenum, the total of manganese and molybdenum lying in the range from 9% to 16%, from 0.01% to 0.08% carbon, from 0.01% to 0.35% nitrogen, up to about 1% silicon, up to 1% vanadium, up to 0.03% boron, up to 0.06% zirconium, and the balance iron with, in some cases, small amounts of additives and small amounts of incidental impurities, the F(c) value of the composition being greater than 14 and the  $\phi(c)$  value lying in the range from 1 to 3.75. The composition functions F(c) and  $\phi(c)$  will be defined hereinafter.

A preferred range of composition for the fully austenitic weldable alloys of this invention is, by weight, from 14% to 18% chromium, from 15% to 26% nickel, from 9%

to 14% manganese, from 1% to 3% molybdenum, the total of manganese and molybdenum lying in the range from 12% to 15%, from 0.01 to 0.06% carbon, from 0.01% to 0.25% nitrogen, up to about 0.6% silicon, up to 1% vanadium, up to 0.02% boron, up to 0.04% zirconium, and the balance iron and small amounts of incidental impurities, the F(c) value of the composition being greater than 14 and the  $\phi(c)$  value lying in the range from 1 to 3.75.

10 An austenitic, highly weldable alloy within the broad range defined above, which is suitable for many conventional stainless steel applications as well as for cryogenic applications, comprises, by weight, from 14% to 18% chromium, from 18.5% to 22% nickel, from 8% to 13% manganese, from 1.0% to 3% molybdenum, the total of manganese and molybdenum lying in the range from 11% to 16%, from 0.01% to 0.06% carbon, from 0.01% to 0.09% nitrogen, from 0.08% to 1% silicon, and the balance iron except for small amounts of incidental impurities, the F(c) value of the composition being greater than 14 and the  $\phi(c)$  value lying in the range from 1 to 3.75. An alloy similar to that just described, but containing from 0.10% to 0.25% nitrogen is especially useful as a high strength, weldable, austenitic stainless steel at 20 cryogenic temperatures.

25 A high strength austenitic weldable stainless steel alloy of this invention comprises, by weight, from 14% to 18% chromium, from 18.5% to 22% nickel, from 8% to 13% manganese, from 1.0% to 3% molybdenum, the total of manganese and molybdenum lying in the range from 11% to 16%, from 0.15% to 0.5% vanadium, from 0.002% to 0.03% boron, from 0.002% to 0.06% zirconium, from 0.1% to 0.35% nitrogen, from 0.01% to 0.06% carbon, up to about 0.6% silicon and the balance iron and small 30 amounts of incidental impurities, the F(c) value of the composition being greater than 14 and the  $\phi(c)$  value lying in the range from 1 to 3.75.

35 A principally austenitic, highly weldable stainless steel alloy of this invention, having from 2% to 10% delta ferrite therein to increase resistance to hot-cracking and hot-tearing and which is especially suitable for castings and for welding electrodes, comprises, by weight, from 14% to 18% chromium, from 5% to 15% nickel, from 8% to 13% manganese, from 1% to 3% molybdenum, the total of manganese and molybdenum lying in the range from 11% to 16%, from 0.01% to 0.08% carbon, from 0.01% to 0.09% nitrogen, from 0.08% to 1% silicon and the balance iron except for small amounts of incidental impurities, the F(c) value of the composition being from 7.5 to 50 11.5 and the  $\phi(c)$  value lying in the range from 1 to 3.75.

45 Stabilizing additions of from 0.25% to 1.5% total of columbium and/or titanium may be added to the alloys of this invention.

50 Larger amounts of titanium may be employed to develop precipitation hardening. Thus, a further alloy of this invention is a precipitation hardenable, austenitic, weldable stainless steel alloy, comprising, by weight, from 14% to 18% chromium, from 15% to 30% nickel, from 9% to 14% manganese, from 1% to 3% molybdenum, the total of manganese and molybdenum lying in the range 11% to 16%, from 1.5% to 2.5% titanium, from 0.01% to 0.06% carbon, from 0.01% to 0.06% nitrogen, up to about 0.4% silicon, up to 0.05% vanadium, up to 0.015% boron, up to 0.03% zirconium, and the balance iron and small amounts of incidental impurities, the F(c) value of the composition being greater than 14 and the  $\phi(c)$  value lying in the range from 1 to 3.75.

55 In general the alloys of this invention are characterized by good resistance to hot-cracking and hot-tearing as indicated by a CPT test number (hereinafter defined) of less than 11.

60 For the purpose of strengthening these alloys, tungsten and vanadium may be used, in combination with 0.5% to 3.75% molybdenum, in amounts of up to 6.5% tungsten and up to 1% vanadium, such that the "equivalent molyb-

denum" content (defined as actual molybdenum plus one-half the tungsten plus twice the vanadium) lies in the range 0.5% to 3.75%. Molybdenum should be present in the minimum amount of at least 0.5% in combination with manganese to provide substantial resistance to hot-cracking.

In the alloys of this invention, the hot-cracking and hot-tearing resistance approach optimal values when the total of manganese and molybdenum is in the range from 12% to 15%. However, substantial benefits are observed in the range from 11% to 16%, and a manganese molybdenum total of as low as 9% may be tolerated where crack promoters are present only in small quantities.

The impurities phosphorus and sulfur are maintained within limits normal for comparable austenitic stainless steels; that is, 0.04% maximum phosphorus and 0.03% maximum sulfur.

In accordance with this invention a number of considerations enter into the selection of the optimum compositions of these stainless steels depending upon the intended service conditions; for example, at high temperatures, in contact with corrosive liquids or in cryogenic equipment. The properties of importance include strength, oxidation and corrosion resistance, ductility, impact strength, stability in long-time high temperature service, dimensional stability and magnetic permeability at low temperatures. The composition may also be related to the form in which the alloy is used; i.e., wrought, cast, or as welding electrodes, and to the thickness and rigidity of the elements being joined. This invention is directed primarily to a new family of stainless steels which have exceptional resistance to hot-cracking and hot-tearing when welded or cast. These and other factors that are necessary to define the composition requirements for various applications of the stainless steel alloys of this invention are discussed in part in the following sections under appropriate headings.

#### HOT-CRACKING

In order to provide a technique for the convenient quantitative evaluation of the hot-tearing and hot-cracking characteristics of alloys, I have developed the Cast Pin Tear test, hereinafter referred to as the CPT test, which has been fully described in the Welding Journal, volume 38, April 1959, pages 176-S to 181-S. In brief, the CPT test involves casting small samples of an alloy in a series of copper molds graduated in size under conditions which impose a tensile strain on the sample as the mold expands and as the casting contracts during solidification and cooling. The geometry of the particular mold that will produce a certain degree of hot-cracking provides a means of classifying alloys in order of merit or of predicting service performance.

From an examination at a suitable magnification of the surface cracking of the pins after cooling, the cumulative percentage of circumferential cracking (cracking index) is determined and plotted against arbitrary mold numbers as illustrated in FIG. 1 to provide a measure of the susceptibility of the alloy to cracking. The molds are graduated so as to serially progress in relatively regular steps from long, slender molds to short, heavy molds. The long slender molds (of the aforementioned series) which have the smaller arbitrarily assigned numbers produce severe cracking, whereas the short, heavy-walled molds which have the larger arbitrarily assigned numbers crack the pin less severely, or not at all.

The results of the CPT test have been found to have good correlation with the performance of weld deposits in actual welds. It is not difficult to understand the correlation found between the test results and the actual cracking observed in alloys cooled from the molten state, because the CPT test is based on the resistance to cracking of a cast structure as it solidifies. Although the ability to predict cracking behavior in the heat-affected zone of a wrought alloy during welding from the same

test results is not nearly as obvious, the CPT tests have been found to correspond to actual welding experience and to correlate with certain results of the RPI test, as will be explained more fully below.

One technique currently used to predict the weldability of wrought stainless steel is Rensselaer Polytechnic Institute (RPI) hot ductility test, described in "Further Studies on the Hot Ductility of High Temperature Alloys," Welding Research Council Bulletin Series, Number 33, February 1957. In this test,  $\frac{1}{4}$  inch diameter specimens of an alloy are heated, by passing a large electric current through them, through a time-temperature cycle that simulates conditions in the heat-affected zone of a weld. When the specimens are pulled at different temperatures of this cycle, it is found that heating close to the melting point has damaged the material, as evidenced by a decrease in its ductility on cooling compared to the ductility measured at equivalent temperatures on heating.

A correlation has been established between the cracking susceptibility of stainless steels as measured by the CPT test and the performance in an RPI type hot ductility test, when the maximum temperature on heating is that at which the strength drops to zero. Without going into the details of a procedure not a part of this invention, it should be understood that it is possible to predict the behavior of stainless steels in the heat-affected zone of the base metal from CPT test results. Although other factors, such as prior thermal and mechanical history of the base metal may influence heat-affected zone cracking, it appears that the primary factor is the alloy composition. Summing up, the CPT test may be used to evaluate austenitic stainless steels for crack resistance in castings, weld metal, and base metal adjacent to welds.

By means of the CPT test, I have evaluated the individual effects of many different alloying elements on the cracking of chromium-nickel stainless steels. The general nature of the test results may be seen in FIG. 1 where the data for a ternary iron-chromium-nickel alloy are graphically presented. The cracking index, or cumulative percentage of circumferential cracking in any one specimen for this alloy ranges from 0 to nearly 180. A cracking index of 40 has been found to be convenient for the purpose of comparison of alloys. It will be noted that the ternary alloy tested in FIG. 1 has a cracking index of 40 at mold number 11. With this in mind, it is interesting to observe FIG. 2 in which the effects of various alloying additions on the ternary alloy of FIG. 1 are set forth in terms of mold number at a cracking index of 40, as a measure of the resistance to hot-tearing and hot-cracking. The smaller the mold number, the more resistant the alloy is to hot-cracking. A high nickel content of 20% was purposely selected for the base composition in this study so that even with substantial additions of "ferrite formers" such as chromium, molybdenum, vanadium and tungsten, the alloy would remain fully austenitic as cast and the effects of the individual alloying elements would not be obscured by variable amounts of delta ferrite in the structure.

FIG. 2 clearly demonstrates that each element exerts an individual effect on the hot-cracking characteristics of the basic alloy which, in many cases, is substantially different from that of the other elements tested. For example, manganese, molybdenum, tungsten and chromium materially increase the resistance to cracking, each to a different degree. On the other hand, copper, silicon, columbium and titanium have a pronounced deleterious effect, each to a different extent. Copper in amounts of less than 0.25% may be found in these alloys since small amounts are often present in scrap. Cobalt and vanadium are almost identical in their results, as far as cracking is concerned, and do not appear to be either beneficial or deleterious. Hence, cobalt may be substituted for equal amounts of nickel up to at least 5% with some beneficial effect on the characteristics of my alloys. Nickel shows only a slight detrimental effect.

Similar information to that of FIG. 2 is presented with respect to certain other elements in FIG. 3. It should be noted that the horizontal scale indicating the amounts of the elements covers only up to 0.25% whereas in FIG. 2 the scale for alloying elements went up to 5%. It is quite apparent that even as little as 0.01% of boron is highly detrimental. Also zirconium and hafnium, in amounts of 0.1%, greatly impair the cracking resistance of the alloy. Nitrogen, in contrast, reduces hot-cracking.

From other tests made, the beneficial or detrimental effects of the additives shown in FIGS. 2 and 3 for the 16% chromium, 20% nickel, balance iron alloys, have been determined to be similar for stainless alloys having other proportions of nickel, chromium, manganese, molybdenum and iron.

As a guide in correlating CPT test results with practice, it has been found that most casting and welding applications are satisfied by an alloy having the crack resistance indicated by a CPT mold number of 8 to 10 for a cracking index of 40. Alloys having CPT mold numbers of 10 or 11 are very useful alloys having many applications. Alloys having a CPT mold number higher than 12 or 13 are only marginally applicable, for cracking is common, and serious difficulties may arise in casting and welding. It is in this range above 12 or 13 that many prior art fully austenitic alloy compositions are found.

Because of the improvement in resistance to hot-cracking I found for manganese additions up to 5% (FIG. 2), I decided to thoroughly investigate the effect of manganese on hot-cracking of iron-chromium-nickel alloys. The results of this study are summarized graphically in FIG. 4. For this work, the chromium content was held constant at approximately 16% while the nickel content ranged between 14% and 20%. The amount of nickel in the alloy assured a fully austenitic structure without dependence on the manganese content. In the graph, the CPT test mold numbers for cracking indices of 40 and zero are plotted against the manganese content, which is varied over the wide range shown. It will be noted that the beneficial effect of manganese on the alloy reaches a maximum at about 14%, and outstanding crack resistance is obtained in the range of 11% to 16% manganese, but that the slopes of the curves are such that substantial beneficial effect extends to the limits of the range 7.5% to 18% manganese. This range of manganese content includes quaternary compositions having higher resistance to cracking than any other quaternary fully austenitic stainless steel containing iron, chromium, and nickel. In the alloys of this invention, the manganese, which has very little effect on delta ferrite formation as will be shown later, is not relied upon to provide the austenitic or face-centered-cubic crystal structure, since that is the function of the nickel addition; the manganese is present primarily to reduce the susceptibility to cracking.

Finally, in the course of investigating the effects of various alloying additions for the purpose of increasing the strength of Fe-Cr-Ni-Mn alloys, it was discovered that not only did molybdenum increase the strength considerably, as might have been anticipated from the prior art, but it furthermore actually reduced susceptibility to hot-cracking. In FIG. 5 CPT test data are plotted from a large number of fully austenitic alloy samples containing approximately 16% chromium and from 14% to 20% nickel in which the manganese and molybdenum contents have been varied over a wide range. As the data are presented in FIG. 5, contours of equal amounts of cracking have been drawn. Compositions having a mold number of about 8.5 or smaller in FIG. 5 are characterized by a resistance to cracking sufficient to permit casting of shapes and welding of restrained joints of heavy sections of nearly all usual types or forms without microfissuring in welds or castings, or base-metal cracking in the heat-affected zone of welds.

With respect to these austenitic iron-chromium-nickel-manganese-molybdenum alloys, it will be observed in FIG. 5 that the greatest resistance to hot-cracking occurs at about 1.5% molybdenum and 12% manganese. Excellent resistance to hot-cracking is exhibited by alloys containing, as preferred ranges, from 1% to 3% molybdenum, and from 9% to 1% manganese. If an alloy having greater strength is desired, improved strength can be obtained by further increasing the molybdenum content, but the increase of molybdenum produces slightly increased susceptibility to hot-cracking. In order to minimize the hot-cracking characteristic in alloys particularly suitable for welding, and having molybdenum in amounts greater than 1.5%, it is preferred to decrease the manganese content by 1% for each 1% increase in molybdenum. Thus, for example, at 3.75% molybdenum it is preferred to use 9.75% manganese. Stated more generally, the minimum susceptibility to hot-cracking at a given molybdenum content is obtained when the total of manganese and molybdenum amounts to from about 12% to 15% by weight, of the alloy. These five component compositions have an exceptional combination of strength and resistance to microfissuring or cracking. Also, equally good alloys are produced by wholly or partially substituting tungsten for the molybdenum, using two parts by weight of tungsten for each part of molybdenum it replaces. For example, in Table VI, in which numerous examples of the alloys of this invention appear, several alloys are listed in which tungsten is substituted for part or all of the molybdenum. These alloys have equally good resistance to hot-cracking because, as shown in FIG. 2, tungsten as well as molybdenum reduces the hot-cracking susceptibility of stainless steels. However, since the tensile and creep properties of the steels of this invention, containing all or part tungsten are not significantly better than those containing only molybdenum, and since tungsten is more expensive than molybdenum per pound and twice as much is needed to produce an equivalent effect, I prefer to use molybdenum alone in my steels for economic reasons. Vanadium does not appreciably affect the hot-cracking characteristics of my steels.

#### STRENGTH

It has been a common practice in the prior art to add various amounts and proportions of molybdenum, tungsten and vanadium to stainless steels to increase the strength. At the lower composition levels these elements act mainly as solid solution strengtheners; but, at higher levels, precipitates form during heat treatment or during elevated temperature testing. I have found in these types of stainless steel alloys that creep and rupture strength increase in an approximately linear manner from 0 up to about 8% equivalent molybdenum, defined as

$$\text{percent Mo} + \frac{(\text{percent W})}{2} + 2(\text{percent V})$$

However, full advantage cannot be taken of this strengthening mechanism because of other side effects on equally important characteristics of the alloys. For example, we have just seen that molybdenum should be kept in the range of about 1% to 3% for optimum resistance to hot-cracking. We must also consider the effects of the content of molybdenum, tungsten, vanadium and other elements on oxidation resistance, stress-rupture ductility and impact strength after long-time aging.

#### OXIDATION RESISTANCE

During high temperature solution heat treatment of these alloys or several thousand hours of aging at 1500° F. and 1350° F., I have observed that, at the preferred chromium content of 16%, the molybdenum should be kept below 4% and vanadium below 0.5% (when it is present in combination with some molybdenum) in order to avoid severe oxidation which can assume the propor-

tions of catastrophic oxidation if these limits are exceeded by an appreciable amount. Tungsten also contributes to rapid oxidation, but greater percentages are required for an equivalent effect. In order to provide a greater margin of safety against this phenomenon, I prefer to keep the molybdenum content below 3.75% and vanadium below 0.35% in alloys for most high temperature applications. Vanadium may be as high as 1%, however, for service temperatures below about 1200° F.

#### STRESS RUPTURE DUCTILITY

Insofar as rupture ductility is concerned in wrought materials, this increases along with strength to a maximum at about the level of 4% molybdenum (or its equivalent) and thereafter decreases. The increased ductility is believed to be due to an optimum amount and distribution of precipitate which forms as beads and plates along the grain boundaries to block boundary sliding. Too little precipitate allows the grain boundaries to slip and fractures occur at junctures between three grains. On the other hand, a continuous film of the brittle sigma phase is detrimental and reduces ductility. In cast structures with a lower amount of grain boundary area per unit volume, the molybdenum content should be below 4%. Actually, the whole composition balance of the alloy is related to the ductility and impact strength.

#### IMPACT STRENGTH

One of the primary distinctions between my invention and the prior art is the discovery in the field of austenitic stainless steels of the need for control of nickel at a higher level than has been recognized as necessary. The literature contains many references illustrating how fully austenitic stainless steels can be produced by substituting one or more of the elements manganese, carbon and nitrogen for all or a major part of the nickel. The aim of many of these developments has been to find a cheaper steel that contains no delta ferrite as cast and whose martensite formation temperature has been lowered to approximately room temperature or below. Manganese, carbon and nitrogen do act as substitutes for nickel in these respects. On the other hand, there is a major difference between these elements and nickel with respect to the high temperature stability of the alloys. Carbon and nitrogen do not appreciably affect the sigma forming characteristics of an alloy, whereas manganese actually promotes sigma formation, in contrast to nickel which tends to suppress it, as will now be shown. Thus, many of the prior art alloys containing high manganese, high carbon and/or nitrogen and low nickel content experience rapid deterioration of impact strength upon aging in elevated temperature service.

In connection with the effect of various alloying additives upon the impact strength of the alloys of this invention, a great number of alloys were investigated and tested after accelerated aging by a simplified impact test, the results of which could be correlated with conventional Charpy test results. In these tests, aging was conducted at 1500° F. for times up to 1000 hours. This condition was taken to simulate the effects of the much longer times encountered at service temperatures which are usually in the range of 1000 to 1200° F. Alloy samples were prepared by levitation melting in an argon atmosphere and 20 gram tapered specimens about 1/4 inch in diameter were cast in copper molds. After aging times of zero, 17, 100 and 1000 hours at 1500° F., the cast specimens were notched half-way through with a hacksaw, held in a vise, and subjected to a simplified impact test. Using the arrangement shown in FIG. 6, from 1 to 20 blows of a one and one-half pound hammer were required to break the notched pins or bend them to a 90° angle. The bend angle at fracture was the value most easily correlated with conventional Charpy test results. FIG. 7 shows the typical curves obtained by this technique for an alloy containing 20% nickel, 10% man-

ganese, 3% molybdenum, 0.1% silicon, chromium in various amounts from 12% to 22% and the balance iron. An alloy containing 16% chromium, 20% nickel, 10% manganese, 2% molybdenum, 0.1% silicon, the balance iron, was used as a base to determine the effects of additions of tungsten, vanadium, columbium, titanium and silicon. In a similar way, with slightly different bases, the effects of chromium, nickel, cobalt, manganese and molybdenum additions were evaluated. These results can be summarized in the form of an equation which reduces the composition of an alloy within the scope of this invention to a single variable  $\phi(c)$  which is uniquely related to the impact properties after aging (alloy components in weight percent).

$$15 \quad \phi(c) = 0.55(Cr-16) + 0.25(Mn-10) + 0.6Si + Mo + V + Ti + 0.55W + 0.7Cb - 0.11(Ni-20) - 0.087Co$$

The larger the value of  $\phi(c)$  the more precipitate was found in the structure after aging. This precipitate, which in large amounts seriously embrittles the alloy, is believed to be the sigma phase. If the 1000 hour notched impact bend angles at fracture for all these alloys are plotted in one graph against  $\phi(c)$ , the results lie within a relatively narrow band as shown in FIG. 8. Carbon and nitrogen up to 0.2% do not appreciably change this relationship. It has been found that in order to have good stress-rupture ductility,  $\phi(c)$  should be greater than about 1.0 and less than 4.0 and to avoid severe loss of impact strength on aging in high temperature service,  $\phi(c)$  should be less than 3.75 and preferably less than 3.0.

#### STABILIZING ADDITIONS

Since the problem of preventing intergranular corrosion of stainless steels in some applications is a serious one, carbide stabilizers such as titanium or columbium are frequently added, in minimum amounts of about 8 and 10 times the carbon, respectively, to stainless steels to prevent intergranular precipitation of chromium carbides with subsequent accelerated corrosion.

Columbium is also effective in increasing strength at high temperature so that smaller ratios of this element may be added where corrosion resistance is not a primary consideration. Small additions of titanium tend to increase hot ductility (see Table XXIV and the text associated therewith) and may be made even in cases where corrosion resistance is not of primary importance. Much larger quantities of titanium in the range of 1.5% to 2.5%, by weight, may be added to obtain precipitation hardening in the alloys of this invention, and this will be discussed in detail hereafter.

It was previously shown in FIG. 2 that titanium and columbium seriously increase the susceptibility to hot-cracking of a chromium-nickel stainless steel. The CPT test was again used to evaluate the effects of these elements in alloys with preferred amounts of manganese and molybdenum and both with and without delta ferrite, as presented in Table I.

Table I

60 EFFECTS OF ALLOYING ELEMENTS AND DELTA FERRITE ON SUSCEPTIBILITY OF STAINLESS STEELS TO HOT-CRACKING

| 65                                 | Composition, Weight Percent, Balance Iron | Percent Delta Ferrite As Cast | CPT Test Mold No. for Cracking Index=40 |
|------------------------------------|-------------------------------------------|-------------------------------|-----------------------------------------|
| 16 Cr, 20 Ni                       | 0                                         | 11.0                          |                                         |
| 16 Cr, 20 Ni + 0.75 Ti             | 0                                         | 13.5                          |                                         |
| 16 Cr, 20 Ni + 1 Cb                | 0                                         | 13.0                          |                                         |
| 16.4 Cr, 14.9 Ni, 10.6 Mn          | 0                                         | 8.2                           |                                         |
| 16 Cr, 14.5 Ni, 11 Mn, 2 Mo        | 0                                         | 8.0                           |                                         |
| 16 Cr, 14.5 Ni, 11 Mn, 2 Mo + 1 Ti | 0                                         | 10.4                          |                                         |
| 16 Cr, 14.5 Ni, 11 Mn, 2 Mo + 1 Cb | 0                                         | 10.2                          |                                         |
| 16 Cr, 10 Ni, 11 Mn, 2 Mo          | 7.3                                       | 7.5                           |                                         |
| 16 Cr, 10 Ni, 11 Mn, 2 Mo + 1 Ti   | 10.4                                      | 9.5                           |                                         |
| 16 Cr, 10 Ni, 11 Mn, 2 Mo + 1 Cb   | 6.6                                       | 9.5                           |                                         |

The relationship of the carbide stabilizers to the hot-cracking properties is also found to hold true in the iron-chromium-nickel-manganese-molybdenum alloys, where it is clear that titanium and columbium significantly increase the hot-cracking tendencies. It is important to note, however, that because of the generally low susceptibility to hot-cracking that has been discovered in the iron-chromium-nickel-manganese-molybdenum alloys with or without tungsten and vanadium, it is possible to employ either titanium or columbium as a stabilizing element in substantial quantities from 0.25% to 1% or slightly higher and still produce alloys which have lower susceptibility to hot-cracking than stainless steels currently in use, and which are sufficiently resistant to cracking to be welded in heavy sections and to be cast into complex shapes. As shown in Table I, even with 1% titanium or 1% columbium, the CPT test mold numbers are 9.5 to 10.4 for such alloys, actually less than the mold number of 11 for the 16% chromium-20% nickel base composition. Without manganese in the alloys, the mold numbers reach the highly undesirable values of 13.5 and 13 when 0.75% titanium and 1% columbium are present.

#### FERRITE CONTROL

The discussion of this new class of stainless steels would be incomplete without some reference to the effects of delta ferrite and methods of controlling ferrite within specified limits or avoiding it in alloys where a fully austenitic structure is desired. In the prior art the conventional means for decreasing the hot-cracking of austenitic stainless steels, on casting complex shapes in a foundry or on welding restrained joints, has been the preparation of steel castings or weld deposits whose cast structures contain a controlled percentage of delta ferrite. In the alloys of this invention, likewise, improved resistance to cracking can be obtained when from 2% to 10% of the total volume of the cast alloy is delta ferrite. However, since delta ferrite is known to accelerate the formation of the brittle sigma phase in alloys during elevated temperature service, it was a primary object of this invention to disclose alloys so resistant to hot-cracking that sound castings and weld deposits could be made that were fully austenitic.

The methods for obtaining a fully austenitic structure or for controlling the amount of delta ferrite in cast alloys and weld deposits of stainless steels are well understood in the prior art. In general, the amounts of chromium and nickel in the alloy are the variables most usually controlled, but other additives in the alloy will also exert an effect upon the phase relationships which must be taken into consideration. For example, if strength and/or corrosion characteristics dictate the levels of solid solution hardeners (molybdenum, tungsten, and vanadium) and stabilizers (titanium and columbium) desired, and melting practice produces a certain level of carbon and nitrogen, if deoxidation yields about 0.5% silicon, there are only chromium, nickel, and manganese left to affect the structure. Since chromium must exceed about 14% to give the steels their stainless characteristics, and manganese has little effect on the amount of delta ferrite (as will be apparent from the following), the primary control over the structure resides in the selection of the nickel content.

Five factors enter into the selection of the optimum nickel content for fully austenitic alloys of this invention:

- (1) Because nickel increases the hot-cracking susceptibility by about 0.5 CPT test mold number for every 5% excess nickel, nickel should be kept low.
- (2) In wrought products it is desired to keep delta ferrite out of the cast ingot or wrought material in order to maintain good workability. Hence, nickel should be high enough to insure a fully austenitic structure.
- (3) When highly restrained joints are welded with a

5 ferrite-containing electrode, if the nickel content of the base metal is too high, dilution of the weld bead by the base metal will decrease or eliminate the delta ferrite from the weld and may cause hot-cracking. From this standpoint the base metal should be as low in nickel as items (2) and (4) will permit.

10 (4) In high temperature service, nickel counteracts the sigma forming tendencies of Cr, Mn, Mo, W, V, Si, Cb and Ti, so the nickel content should be high enough to prevent serious embrittlement.

15 (5) Finally, from practical considerations, higher nickel than needed for items (2) and (4) is uneconomical and wasteful.

20 For the composition ranges covered by this invention I have determined the nickel equivalents of the various additives so that a fully austenitic alloy or one having a predetermined delta ferrite content can be obtained as desired. The high level of manganese in the alloys of the present invention might be expected to introduce a variable not met with in the prior art. The effects of nickel on the amount of delta ferrite in alloys containing 16% chromium and 11% or 14% manganese plus additions of titanium, columbium, vanadium, tungsten, silicon, nitrogen and molybdenum are shown in Table II.

25 *Table II*

30 EFFECTS OF VARIOUS ELEMENTS ON MICROSTRUCTURE OF CAST STAINLESS STEELS

| Principal Alloying Elements, Weight Percent, Balance Ni and Fe | Percent Nickel for the Indicated Microstructures |                    |                  |
|----------------------------------------------------------------|--------------------------------------------------|--------------------|------------------|
|                                                                | 10% Delta Ferrite                                | 2.5% Delta Ferrite | Fully Austenitic |
| 16 Cr, 14 Mn, 1.75 Ti                                          | 9                                                | 14                 | >15              |
| 16 Cr, 14 Mn, 1.62 Cb                                          | 7                                                | 11                 | >11.5            |
| 16 Cr, 14 Mn, 2.98 V                                           | 14.5                                             | 16.7               | >17              |
| 16 Cr, 14 Mn, 4.54 W                                           | 10                                               | 13.3               | >14              |
| 16 Cr, 14 Mn                                                   | 4.5                                              | 10.7               | >11.5            |
| 16 Cr, 14 Mn, 2.89 Si                                          | 7.5                                              | 12.0               | >13              |
| 16 Cr, 14 Mn, 0.11 N                                           | 3.5                                              | 6.7                | >8               |
| 16 Cr, 11 Mn, 2 Mo                                             | 7                                                | 13.3               | >14              |

45 From these and similar determinations it has been found that the effects of the alloying elements to be as follows in producing delta ferrite in my steels, if nickel is assigned an austenite forming tendency of +1 for each weight percent nickel (a minus sign indicates a tendency to form delta ferrite):

50 *Table III*

55 AUSTENITE(+) AND DELTA FERRITE(-) FORMING TENDENCIES OF ALLOYING ELEMENTS

|    |       |
|----|-------|
| V  | -2.0  |
| Ti | -1.8  |
| Mo | -0.8  |
| Cr | -0.7  |
| W  | -0.5  |
| Si | -0.4  |
| Cb | -0.1  |
| Mn | +0.02 |
| Ni | +1.0  |
| C  | +37   |
| N  | +37   |

70 Using the above values, the following equation has been derived which enables one to predict the microstructures of castings and weld deposits of alloys of this invention. When the composition function,  $F(c)$  in the following equation, exceeds about 13 to 14 the alloy will be substantially austenitic, whereas when it lies between 7.5 and 11.5 the alloy will contain about 10% to 2%

delta ferrite. The smaller values of  $F(c)$  correspond to larger amounts of delta ferrite. Thus, for example, the 16Cr-10Ni-11Mn-2Mo-1Cb alloy in Table I has an  $F(c)$  value of 8.9 and contains 6.6% delta ferrite, whereas heat number 7392 in Table V has an  $F(c)$  value of 13.5 and is fully austenitic as cast.

$$F(c) = (\text{percent Ni}) + 0.02 (\text{percent Mn}) + 37 (\text{percent C} + \text{percent N}) - 2.0 (\text{percent V}) - 1.8 (\text{percent Ti}) - 0.8 (\text{percent Mo}) - 0.7 (\text{percent Cr-16}) - 0.5 (\text{percent W}) - 0.4 (\text{percent Si}) - 0.1 (\text{percent Cb})$$

Of particular interest in the application of the present invention is the unexpected discovery that manganese has practically no effect on the austenite-delta ferrite limits in cast alloys (nickel is 50 times more effective than manganese). However, manganese helps suppress the transformation of austenite to martensite if the total alloy content of chromium and nickel is low, as for example, at 16% chromium and 10% nickel.

Another item of interest is the very small effect of columbium per se on the amount of delta ferrite. There is, however, an interaction between (columbium and/or titanium) and (carbon and/or nitrogen) such that if both are present in substantial amounts carbon and nitrogen appear to be removed from solution as carbides and nitrides and delta ferrite appears in the microstructure at a somewhat higher nickel content than predicted by the equation.

The effect of the nickel content and the delta ferrite content on the hot-tearing of stainless steels is illustrated clearly in FIG. 9. In that figure, cracking index in the number 6 CPT test mold has been plotted against nickel content for constant chromium of 16% and manganese contents of 0% and 14%. In the fully austenitic range, cracking for both alloys decreases gradually as nickel decreases from 20% to 11%. However, as delta ferrite appears in the as-cast pins, cracking decreases at first abruptly and then more slowly as nickel decreases. It is significant that even with alloys containing delta ferrite, a substantial and unexpected decrease in susceptibility to hot-tearing is produced by the addition of 14% manganese.

The hot-tearing characteristics of a molybdenum-containing alloy were determined for alloys containing 16% chromium, 11% manganese and 2% molybdenum. The nickel content of these alloys was varied from 6% to 20%. As in the alloys which did not contain molybdenum, an especially low susceptibility to hot-tearing was found below about 11% nickel; this corresponds to a delta ferrite content of about 7% by volume in the as-cast structure.

In Table I, alloys of iron-chromium-nickel-manganese which have been solid-solution hardened with molybdenum and stabilized with either titanium or columbium, and which contain significant amounts of delta ferrite may be compared with similar alloys which do not contain delta ferrite, as to these hot-tearing properties. It will be observed that improvements in resistance to hot-tearing are effected by the presence of the delta ferrite phase.

#### STRENGTH—CARBON AND NITROGEN

Since the potential strengthening due to increasing the amounts of molybdenum, tungsten and vanadium is limited by the considerations of oxidation resistance and impact strength after aging, mentioned above, it is clear that if still higher strength alloys are needed, additional alloying elements and strengthening mechanisms must be relied upon. In the prior art, carbon and nitrogen individually and in combination have been used many times to strengthen stainless steel. However, based on the hot-cracking consideration and the effect of carbide precipita-

tion on impact strength, it is necessary to keep the carbon content low in the steels of this invention, that is, generally below .08% and preferably below .06%. Accordingly, an increase in carbon content is not a feasible method of increasing strength in these alloys. On the other hand, FIG. 3 shows nitrogen to have the beneficial effect of reducing hot-cracking. Table IV and FIGS. 10 and 11 show that Heat No. 7470 with 0.13% N has significantly higher stress rupture and creep strength than the heats of lower nitrogen content.

Table IV  
STRESS RUPTURE AND CREEP PROPERTIES

| Heat No. | Percent Nitrogen | 1,200° F.-1,000 Hr.    |                    | Stress for .01% per hour minimum creep rate at 1,200° F., p.s.i. |
|----------|------------------|------------------------|--------------------|------------------------------------------------------------------|
|          |                  | Rupture Stress, p.s.i. | Percent Elongation |                                                                  |
| 7392     | .016             | 15,000                 | 55                 | 14,000                                                           |
| 7431     | .019             | 16,500                 | 32                 | 16,000                                                           |
| XMM2054  | .040             | 19,000                 | 75                 | 15,000                                                           |
| 7454     | .041             | 20,000                 | 76                 | 17,000                                                           |
| 7470     | .13              | 23,000                 | 20                 | 22,000                                                           |

Yield and tensile strengths are higher as well.

Nitrogen contents in excess of about 0.15% are not desirable in the simple Fe-Cr-Ni-Mn-Mo steels, because a lamellar grain boundary precipitate, which has a detrimental effect on ductility, forms during high temperature service. It is clear then, that moderate increases in nitrogen content will increase strength without serious detrimental effects.

#### LOW TEMPERATURE AUSTENITE STABILITY OF WELDABLE STAINLESS STEEL

The weldable steels of this invention are useful for cryogenic applications either as castings, wrought products or welding electrodes. The particular advantage of these alloys over most conventional stainless steels is that the austenite is completely stable when cooled to or even when deformed at temperatures approaching absolute zero, thus providing a material with a high degree of dimensional stability and one which remains completely non-magnetic. Ball valves for handling liquefied gases and hydrogen bubble chambers are examples of applications requiring these characteristics.

A tensile specimen machined from a large commercial casting was tested at -423° F. The fractured specimen which had elongated 42% and had 30% reduction of area showed no detectable ferrite as measured at room temperature. This specific casting had a composition of 16.2% Cr, 16.5% Ni, 11.1% Mn, 0.42% Si, 3.02% Mo, 0.04% C, 0.008% S, 0.024% P and balance iron. However, this test left unanswered the question of whether martensite would have formed if the composition was slightly different, the test temperature lower or the deformation more severe.

In order to determine the effect of these variables, a series of small chill castings was made with variable nickel content and with the remaining elements held constant at 16% Cr, 11% Mn, 2% Mo, 0.004% C, 0.002% N, <0.03% Si, balance iron. A block of hardened steel and a 1/4" diameter by 1/4" high cylinder of the alloy to be tested were cooled in liquid nitrogen. These were then placed on an anvil and the specimen quickly upset by hammering to 1/8" high. The equivalent ferrite or martensite

as measured at room temperature after this 50% reduction in height of a cylinder at  $-320^{\circ}$  F. was as follows:

| Percent Ni: | Percent Ferrite + martensite |
|-------------|------------------------------|
| 8           | >20                          |
| 9           | 16                           |
| 10          | 13                           |
| 11          | 10.5                         |
| 12          | 7.5                          |
| 13          | 4.7                          |
| 14          | 0.3                          |
| 14.5        | 0                            |

An alloy containing 16% Cr, 14.5% Ni, 11% Mn, 2% Mo, balance iron thus has an  $M_d$  temperature of  $-320^{\circ}$  F. The  $M_d$  temperature is the lowest temperature at which a sample may be deformed without producing martensite. The  $M_d$  temperature is normally about  $600^{\circ}$  F. higher than the  $M_s$  temperature, the temperature at which martensite forms on cooling and thus is a more severe standard of austenite stability. From some similar tests, the effects of changes of Ni, Cr, Mn, Mo, Si, C and N from this base on  $M_d$  would be approximately as follows:

| Element | $\Delta M_d$ / percent increase, ° F. |
|---------|---------------------------------------|
| Ni      | 110                                   |
| Cr      | 55                                    |
| Mn      | 55                                    |
| Mo      | 65                                    |
| Si      | 50                                    |
| C       | 3000                                  |
| N       | 3000                                  |

For example, if the nickel content of the above alloy were increased only 1% to 15.5%,  $M_d$  would be approximately  $-430^{\circ}$  F. With the normal contents of carbon and nitrogen specified in these steels and with nickel greater than 15%, the austenite in the alloys is fully stable down to liquid helium temperatures.

The specification thus far has been devoted primarily to a description of various quantitative relationships which I have discovered that relate the composition of stainless steels to the major characteristics governing their use. These characteristics include hot-cracking, strength, oxidation resistance, stress-rupture ductility, impact strength after long-time aging, corrosion resistance, and control of delta ferrite. These relationships have been used as a guide in determining the types and amounts of additions to make in a novel stainless steel which combines an excellent level of all the above properties, including especially an unexpectedly high resistance to hot-cracking. Reviewing these findings in general terms, I have found that, in the basic composition, a high resistance to oxidation and hot-cracking as well as good mechanical properties are obtained when the chromium content is as high as it can be without giving rise to delta ferrite and too much sigma phase, and when nickel is as low as it can be without similarly producing delta ferrite and sigma. Manganese should be maintained at a high level and in a particular relationship to the molybdenum content. Aluminum, copper and silicon should be maintained at a low level. The solid solution hardeners molybdenum, tungsten and vanadium could be added in relatively large amounts to obtain high rupture strength but must be limited by their effects on oxidation, rupture ductility and impact strength. Molybdenum and tungsten actually increase the resistance to cracking when used in the proper amounts, while vanadium does not adversely affect the cracking characteristics in any amount up to 5%. Of the austenite stabilizers and strengthening elements, carbon and nitrogen, nitrogen is to be preferred over carbon because nitrogen reduces hot-cracking. The carbide stabi-

lizers titanium and columbium increase the susceptibility of the alloy to hot-cracking. Therefore, if a stabilizing addition is used to increase the strength or is required to prevent intergranular corrosion of as-welded structures, or materials heated in the sensitizing temperature range, the amount of titanium or columbium added should be restricted to as low a level as possible, consistent with the requirements. Because carbon is detrimental to hot-cracking and also increases the amount of titanium or columbium needed for stabilization, there are two reasons for keeping the carbon level low. Certain elements, such as boron and zirconium, which are sometimes added to austenitic stainless steels to obtain particular characteristics, are especially potent in increasing hot-tearing and cracking, and, therefore, whenever these elements are added to an alloy in which the hot-cracking property is of special importance, care should be taken to restrict the amount of these elements to the lowest level consistent with attaining the desired result. The effect of hafnium on cracking is similar to that of zirconium.

In partial summary of the major points thus far presented, it has been found that Fe-Cr-Ni alloys with 1.5% Mo and 12% Mn have unusually high and unexpected resistance to hot-cracking. In the preferred range of 12% to 15% (Mn+Mo), molybdenum is limited on the high side by considerations of hot-cracking, oxidation resistance and impact strength to a maximum of about 3.75% and preferably 3.0%. On the low side, resistance to hot-cracking, rupture ductility and strength dictate a lower limit of 0.5% and preferably 1.0% Mo. The broad range of manganese in these particular alloys is 7.5% to 15% and the preferred range is 9% to 14% Mn. If only small amounts of crack promoters are present, the manganese range may be somewhat lower, as for example, 8% to 13%. The broad range of molybdenum is 0.5 to 3.75% in these alloys and the preferred range is 1 to 3%. Tungsten may be substituted for all or part of the molybdenum, but since it is more expensive and provides no additional benefit, molybdenum is preferred. Vanadium is limited to 1% and preferably 0.5% because of oxidation resistance. Columbium may be added in amounts of from 0.25% to 1.5% to stabilize the carbides or increase high temperature strength. Titanium also acts as a carbide stabilizer in the range of 0.25% to 1.5%. Amounts of from about 0.25% to 0.5% or higher produce a marked increase in hot tensile ductility. Finally, in the range of 1.5% to 2.5% titanium the precipitation hardening phenomenon occurs, producing increased strength. Chromium must be at least 14% to provide oxidation and corrosion resistance but should not exceed 20% because this would require too high a nickel content to maintain the composition balance. Almost all of the alloying elements in the steel affect the balance of austenite and ferrite.  $F(c)$  as defined should have a value of 7.5-11.5 if 2-10% delta ferrite is desired in the cast structure. For a fully austenitic structure  $F(c)$  should be greater than about 14. The whole composition also influences the rate of sigma formation and thus the loss of impact strength on long time aging at elevated temperature. Some sigma formation though is desired to increase strength and stress-rupture ductility. The required range for the composition function  $\phi(c)$ , as defined, to meet these objectives is 1 to 3.75 and preferably 1.5 to 3.

A number of alloys were made in the course of these studies which had good resistance to hot-cracking and which incorporated various amounts and combinations of additives. The compositions and CPT test ratings are given in Table V. Compositions of some additional alloys are given in Table VI. Not all of the alloys in these tables are within the scope of this invention as defined by the claims, for they may fail to meet one or more of the requirements set forth in the preceding discussion.

Table V

COMPOSITIONS OF ALLOYS IN WEIGHT PERCENT AND THEIR HOT-CRACKING SUSCEPTIBILITY RATING

| Heat No.             | CPT <sup>1</sup><br>Test<br>Mold<br>No. | Cr   | Ni   | Mn   | Si     | Mo     | W     | V    | Ti   | Cb   | C    | N      | Fe      |
|----------------------|-----------------------------------------|------|------|------|--------|--------|-------|------|------|------|------|--------|---------|
| 7447                 |                                         | 7.8  | (16) | (7)  | (11.5) | (.15)  | (1.5) |      |      |      |      | (.03)  | (.08)   |
| 7392                 |                                         | 8.5  | 16.3 | 14.0 | 12.0   | (0.16) | 1.58  |      |      |      |      | 0.0062 | 0.016   |
| 7393                 |                                         |      | 16.4 | 14.0 | 12.3   | (0.15) | 1.48  |      |      |      |      | (0.01) | (0.015) |
| 7397                 |                                         | 8.5  | 16.4 | 13.8 | 12.1   | 0.2    | 1.57  |      |      | 0.47 |      | 0.050  |         |
| 7403                 |                                         | 8.7  | 16.5 | 13.9 | 11.9   | 0.14   | 1.51  |      | 1.05 |      |      | 0.082  | 0.041   |
| 7405                 |                                         | 9.0  | 16.3 | 14.0 | 12.0   | 0.13   | 1.53  | 0.90 |      |      |      | 0.070  | 0.026   |
| 7408                 |                                         | 8.5  | 17.0 | 16.6 | 15.0   | 0.10   |       |      |      |      |      | 0.006  | 0.055   |
| 7451                 |                                         | 10.2 | (16) | (14) | 10.7   | (0.15) | 2.74  |      |      |      | 0.47 | 0.039  | 0.073   |
| 7410                 |                                         | 9.2  | 16.7 | 15.8 | 14.2   | 0.22   |       | 0.37 | 1.89 |      | 1.32 | 0.014  | 0.021   |
| 7448                 |                                         | 9.0  | (16) | (14) | 10.7   | (0.15) | 2.71  |      |      | 0.14 |      | 0.033  | 0.043   |
| 7411                 |                                         | 8.7  | 16.4 | 15.9 | 14.3   | 0.13   |       | 0.97 |      | 1.15 |      | 0.009  | 0.012   |
| 7440                 |                                         | 9.4  | (16) | (25) | 11.0   | (.15)  |       | 4.60 |      |      |      | 0.006  | 0.016   |
| 7441                 |                                         | 9.6  | (16) | (25) | 11.7   | (.15)  |       |      | 3.21 |      |      | 0.0035 | 0.021   |
| 7431                 |                                         | 8.5  | (16) | (20) | 10.6   | (.15)  | 2.69  |      |      |      |      | 0.0044 | 0.019   |
| 7427                 |                                         | 9.0  | (16) | (22) | 8.93   | (.15)  | 3.88  |      |      |      |      | 0.078  | 0.017   |
| 7432                 |                                         | 9.4  | (16) | (22) | 16.0   | (.15)  | 3.95  |      |      |      |      | 0.0035 | 0.024   |
| 7429                 |                                         | 9.6  | (16) | (20) | 20.1   | (.15)  |       |      |      |      |      | 0.0037 | 0.016   |
| XMM2054 <sup>2</sup> |                                         | 9.0  | 17.1 | 16.0 | 10.5   | 0.28   | 2.74  |      |      |      |      | 0.032  | 0.040   |

<sup>1</sup> Mold No. for Cracking Index=40. Parenthesis ( ) indicates nominal analysis.

2 3,000 pound melt.

Table VI

COMPOSITION OF HEATS, WEIGHT PERCENT (BALANCE FE+IMPURITIES)

| Heat No.        | Cr                | Ni   | Mn   | Si   | C     | N    | Mo   | W    | V   | B     | Zr    | Ti    | Cb  | Ta  |
|-----------------|-------------------|------|------|------|-------|------|------|------|-----|-------|-------|-------|-----|-----|
| 7431            | 16                | 20   | 10.6 | .15  | .0044 | .019 | 2.69 |      |     |       |       |       |     |     |
| 7454            | 16.3              | 17.0 | 9.43 | .21  | .039  | .041 | 2.91 |      |     |       |       |       |     |     |
| 7458            | 16                | 18   | 7.80 | .15  | .031  | .015 | 1.46 |      |     |       |       | .41   |     |     |
| 7459            | 16                | 18   | 7.85 | .15  | .040  | .018 | 1.46 |      |     |       |       | .99   |     |     |
| 7460            | 18                | 18   | 10.3 | .15  | .040  | .023 | 3.64 |      |     |       |       | .41   |     |     |
| 7462            | 16.0              | 17.8 | 7.76 | .16  | .054  | .098 | 1.43 |      | .26 |       |       | 1.15  |     |     |
| 7467            | 15.2              | 16.9 | 9.61 | .32  | .048  | .11  | 2.72 |      |     | .0037 |       | <.03  |     |     |
| 7470            | 16                | 20   | 9.02 | .15  | .037  | .13  | 2.06 |      |     |       |       |       |     |     |
| 7471            | 16                | 20   | 8.92 | .15  | .032  | .11  | 1.39 | .71  | .57 |       |       |       |     |     |
| 7472            | 16                | 20   | 8.32 | .15  | .040  | .074 | 1.36 | .86  | .55 |       |       |       | .41 | .22 |
| 7478            | 16                | 20   | 9.07 | .15  | .036  | .091 | 2.08 |      |     | .0060 |       | (.05) |     |     |
| 7479            | 16                | 20   | 8.95 | .15  | .034  | .12  | 2.03 |      |     | .0045 | .003  | (.05) |     |     |
| 7480            | 16                | 20   | 9.08 | .15  | .033  | .12  | 2.03 |      |     | .0019 | .0098 | (.05) |     |     |
| 7486            | 16                | 20   | 8.80 | .15  | .042  | .058 | 1.16 | .45  | .31 | .0026 | .012  | (.05) | .39 | .12 |
| 7487            | 16.6              | 20.7 | 11.5 | .09  | .035  | .15  | 2.14 |      | .34 | .0060 | .011  | (.05) |     |     |
| 7488            | See Heat No. 7487 |      |      |      |       | .13  |      |      |     |       |       |       |     |     |
| 7489            | 16                | 20   | 8.62 | .15  | .044  | .12  | 2.00 |      | .31 | .0051 | .017  | (.05) |     |     |
| 7530            | 16                | 20   | 8.53 | .15  | .035  | .019 | 2.12 |      | .29 | .010  | .016  | (.05) |     |     |
| 7531            | 16                | 20   | 9.54 | .25  | .030  | .040 | 1.91 | .65  | .29 | .0060 | .049  | (.10) |     |     |
| 7532            | 16                | 20   | 9.32 | .25  | .035  | .044 | 2.18 |      | .29 | .0071 | .005  | (.10) |     |     |
| 7533            | 16                | 20   | 9.91 | .25  | .031  | .053 |      | 1.72 | .29 | .0083 | .003  | (.10) |     |     |
| 7534            | 15.8              | 19.3 | 9.67 | .29  | .026  | .052 | 2.24 |      | .29 | .016  | .044  | <.01  |     |     |
| 7535            | 16                | 20   | 9.45 | .25  | .028  | .045 | 2.24 |      | .25 | .011  | .062  |       |     |     |
| 7571            | 15.0              | 19.7 | 10.4 | .12  | .038  | .19  | 2.25 |      | .26 | .0057 | .012  | (.10) |     |     |
| 7572            | 16                | 20   | 10.6 | .15  | .030  | .23  | 2.23 |      | .25 | .0095 | .013  | (.05) |     |     |
| 7577            | 15                | 19.5 | 8.17 | .096 | .034  | .19  | 2.40 |      | .24 | .012  | .017  | (.05) |     |     |
| VM545           | 16.7              | 20   | 12.6 | <.02 | .017  | .15  | 2.61 |      | .23 | .025  | .012  |       |     |     |
| X MM2216        | 15.9              | 19.7 | 10.1 | .27  | .035  |      | 2.25 |      |     |       |       |       |     |     |
| X MM2264        | 15.9              | 19.7 | 9.37 | .37  | .031  | .056 | 2.13 |      |     |       |       |       |     |     |
| X MM2232        | 16.0              | 20.4 | 9.03 | .37  | .031  | .10  | 2.24 |      | .26 | .007  | .025  |       |     |     |
| 2239            | 16.0              | 19.5 | 8.97 | .31  | .038  | .071 | 2.16 |      | .26 | .004  | .0042 |       |     |     |
| 2240            | 15.9              | 19.4 | 9.02 | .31  | .034  | .094 | 2.11 |      | .26 | .005  | .009  |       |     |     |
| 2265            | 15.7              | 19.8 | 10.6 | .36  | .026  | .16  | 2.22 |      | .26 | .008  | .036  | .06   |     |     |
| 2266 (wire)     | 15.8              | 19.7 | 10.7 | .42  | .024  | .13  | 2.17 |      | .27 | .010  | .043  | .05   |     |     |
| KV101           | 15.7              | 20.0 | 10.3 | .48  | .025  | .13  | 2.32 |      | .28 | .006  | .008  |       |     |     |
| X MM2277 (wire) | 15.9              | 20.2 | 11.6 | .19  | .017  | .14  | 2.32 |      | .30 | .01   | .044  | .017  |     |     |
| 2284            | 15.9              | 20.1 | 11.0 | .20  | .021  | .17  | 2.27 |      | .25 | .007  | .020  | .06   |     |     |

With the information obtained from the series of 25 60 pound heats set forth in Table V it was possible to prepare and study heats of commercial size having preferred compositions. One such heat is identified as XMM2054.

The tensile properties of heat XMM2054 from room temperature to 2200° F. are listed in Table VII. The specimens were cut in the longitudinal direction from a 1½" thick hot-rolled plate which was solution heat treated one hour at 2000° F. There is a minor dip in ductility at about 1350° F. However, since the minimum reduction of area up to 2200° F. is greater than 35%, this wrought alloy is sufficiently ductile to withstand all normal fabrication and service imposed strains, including annealing and stress-relief heat treatment of restrained joints in heavy welded sections.

Table VII

TENSILE PROPERTIES OF HEAT NO. XMM2054 1 1/8" THICK  
HOT-ROLLED PLATE SOLUTION TREATED 1 HOUR AT  
2000° F. AND WATER QUENCHED (STRAIN RATE 750% PER  
HOUR, SPECIMEN 0.357" DIAMETER GAGE LENGTH 1 1/8")

| Test<br>Temp.,<br>° F. | 0.2% Yield<br>Strength,<br>p.s.i. | Ultimate<br>Strength,<br>p.s.i. | Total<br>Elongation,<br>percent | Reduction<br>of Area,<br>percent |
|------------------------|-----------------------------------|---------------------------------|---------------------------------|----------------------------------|
| R.T.                   | 30,300                            | 75,900                          | 61.5                            | 77.5                             |
| 600                    | 20,100                            | 61,100                          | 47.8                            | 70.3                             |
| 1,100                  | 13,000                            | 52,900                          | 49.1                            | 68.9                             |
| 1,350                  | 13,600                            | 36,300                          | 36.9                            | 38.6                             |
| 1,600                  | 12,900                            | 21,400                          | 65.7                            | 52.8                             |
| 1,800                  | 9,600                             | 11,600                          | 75.8                            | 53.1                             |
| 2,000                  | 5,400                             | 7,000                           | 71.2                            | 52.0                             |
| 2,200                  | 3,500                             | 3,800                           | 79.7                            | 87.2                             |

The tensile properties of certain of the other alloys in Table V were determined on  $5/8$ " diameter hot-rolled bars solution treated to give about an ASTM No. 5 grain size. Because of the similarity of these results to the example above, only the properties at room temperature, 1100° F. and 2000° F. are listed in Table VIII. The alloys of this invention generally exhibit excellent tensile ductility up to 2200° F., comparable to the results given in Table VIII.

Table VIII

TENSILE PROPERTIES OF STAINLESS STEELS (STRAIN RATE 750% PER HOUR; SPECIMEN 0.357" DIAMETER, 1 $\frac{1}{2}$ " GAGE LENGTH)

| Heat No. | Test Temp., °F. | 0.5% Yield Strength, p.s.i. | Ultimate Strength, p.s.i. | Percent Elongation | Percent Reduction of Area |
|----------|-----------------|-----------------------------|---------------------------|--------------------|---------------------------|
| 7392     | RT              | 26,800                      | 70,600                    | 62.1               | 78.0                      |
|          | 1,100           | 13,300                      | 47,200                    | 40.8               | 69.3                      |
|          | 2,000           | 4,600                       | 5,600                     | 67.5               | 55.1                      |
| 7403     | RT              | 38,600                      | 87,100                    | 53.3               | 69.4                      |
|          | 1,100           | 20,800                      | 67,800                    | 40.4               | 50.4                      |
| 7405     | RT              | 33,100                      | 79,200                    | 64.0               | 79.5                      |
|          | 1,100           | 16,000                      | 57,000                    | 50.0               | 69.6                      |
|          | 2,000           | 5,500                       | 6,300                     | 51.0               | 46.2                      |
| 7408     | RT              | 29,200                      | 75,200                    | 54.8               | 78.5                      |
|          | 1,100           | 14,300                      | 47,700                    | 39.1               | 55.4                      |
|          | 2,000           | 4,300                       | 5,300                     | 68.9               | 48.6                      |
| 7410     | RT              | 30,000                      | 78,500                    | 50.6               | 69.1                      |
|          | 1,100           | 17,800                      | 59,000                    | 40.2               | 58.4                      |
|          | 2,000           | 5,300                       | 5,800                     | 62.2               | 54.6                      |
| 7429     | RT              | 25,900                      | 72,500                    | 55.0               | 73.9                      |
|          | 1,100           | 14,500                      | 46,600                    | 30.8               | 40.9                      |
|          | 2,000           | 5,000                       | 5,600                     | 39.0               | 31.6                      |
| 7431     | RT              | 29,800                      | 77,600                    | 54.8               | 75.7                      |
|          | 1,100           | 15,500                      | 54,100                    | 45.3               | 68.8                      |
|          | 2,000           | 5,600                       | 6,200                     | 35.0               | 34.3                      |
| 7432     | RT              | 39,500                      | 92,100                    | 46.0               | 66.0                      |
|          | 1,100           | 23,050                      | 63,700                    | 32.9               | 46.0                      |
|          | 2,000           | 6,300                       | 6,300                     | 39.0               | 36.8                      |
| 7440     | RT              | 32,600                      | 82,000                    | 51.6               | 72.4                      |
|          | 1,100           | 18,600                      | 59,400                    | 41.7               | 63.5                      |
|          | 2,000           | 6,200                       | 6,900                     | 34.5               | 29.1                      |
| 7441     | RT              | 32,800                      | 81,600                    | 50.2               | 71.8                      |
|          | 1,100           | 18,500                      | 58,100                    | 36.7               | 53.9                      |
|          | 2,000           | 4,500                       | 5,200                     | 35.9               | 43.1                      |

Heat XMM2054 was successfully worked by the conventional techniques of forging, rolling and wire drawing. The alloy was readily deformed with stiffness similar to commercial stainless steels. There was no tendency to rupture during forging deformations, at various temperatures and degrees of severity.

Results of creep-rupture tests on the alloy heat XMM2054 are presented in Table IX.

Table IX

STRESS-RUPTURE TESTS OF XMM2054 1 $\frac{1}{2}$ " THICK HOT-ROLLED PLATE SOLUTION TREATED 1 HOUR AT 2000° F. AND WATER QUENCHED SPECIMEN 0.505" DIAMETER, GAGE LENGTH 3"

| Test Temp., °F. | Stress, p.s.i. | Rupture Time, hours | Rupture Strain, percent | Reduction of Area, percent | Minimum Creep Rate, Percent per hour |
|-----------------|----------------|---------------------|-------------------------|----------------------------|--------------------------------------|
| 1,050           | 40,000         | 580                 | 19.2                    | 22.4                       | 0.0042                               |
| 1,100           | 27,500         | 900                 | 38.4                    | 36.0                       | 0.022                                |
| 1,200           | 30,000         | 46                  | 61.2                    | 53.5                       | 0.54                                 |
|                 | 25,000         | 143                 | 54.1                    | 60.6                       | 0.13                                 |
|                 | 21,000         | 523                 | 78.7                    | 68.2                       | 0.049                                |
|                 | 18,000         | 1,311               | 94.3                    | 68.9                       | 0.023                                |
|                 | 15,000         | 3,148               | 58.3                    | 55.0                       | 0.010                                |
| 1,350           | 12,500         | 281                 | 21.1                    | 21.9                       | 0.034                                |
| 1,500           | 6,000          | 429                 | 14.3                    | 21.3                       | 0.017                                |
| 1,600           | 4,500          | 277                 | 33.7                    | 27.8                       | 0.050                                |

This type alloy has rupture strength and ductility comparable with the AISI type 316 steel, but it differs from type 316 in being fully austenitic as cast and in weld deposits, the wrought base metal is more resistant to cracking in the heat-affected zone of welds, and the austenite does not transform to martensite even when deformed at cryogenic temperatures.

The 1200° F. stress-rupture and creep properties of certain of the weldable stainless steels of Tables V and VI are summarized in Table IV, which illustrates the effect of nitrogen on strength, and in Table X which shows the effects of various levels and combinations of Mo, W, V, Ti, Cr, C and N.

Table X  
SUMMARY OF 1200° F. STRESS-RUPTURE AND CREEP STRENGTHS OF WELDABLE STAINLESS STEELS

| Heat No. | 1,000 Hour Properties  |                         | Stress for 0.01% per hour Minimum Creep Rate, p.s.i. |
|----------|------------------------|-------------------------|------------------------------------------------------|
|          | Rupture Stress, p.s.i. | Rupture Strain, Percent |                                                      |
| 15       |                        |                         |                                                      |
| 7403     | 22,000                 | 22                      | 29,000                                               |
| 7405     | 17,000                 | 42                      | 15,000                                               |
| 7408     | 12,000                 | 17                      | 11,000                                               |
| 7410     | 18,000                 | 12                      | 28,000                                               |
| 7411     | 22,500                 | 15                      | 23,000                                               |
| 7427     | 21,000                 | 12                      | 21,000                                               |
| 7429     | 10,000                 | 18                      | 10,000                                               |
| 7432     | 14,000                 | 15                      |                                                      |
| 7440     | 15,500                 | 24                      |                                                      |
| 7441     | 17,000                 | 20                      | 20,000                                               |
| 7448     | 19,500                 | 32                      |                                                      |
| 7451     | 26,000                 | 19                      | 34,000                                               |
| 7458     | 20,500                 | 38                      | 21,000                                               |
| 7460     | 20,000                 | 18                      | 18,000                                               |
|          | 20,500                 | 29                      | 23,000                                               |

From these and other data it is possible to draw some conclusions about the effects of different alloying elements on the high temperature strength of these stainless steels. Simple Fe-Cr-Ni-Mn alloys, as illustrated by heats 7403 and 7429, are exceedingly weak with the alloy containing 20.1% manganese (heat 7429) having even lower strength than the alloy with 15.0% manganese (heat 7408). Substantial additions of 4.6% tungsten alone in heat 7440, 3.21% vanadium alone in heat 7441 and molybdenum from about 1.4% to 3.9% in several other alloys produced alloys of intermediate strength. Heats 7448, 7458, 7460, 7459 and 7411 containing increasing amounts of titanium from 0.14% to 1.15% show little or no increase in strength in this titanium range over alloys of similar molybdenum content without titanium. A significant effect of titanium on hot tensile ductility will be discussed later. The three alloys in Table X which have the highest creep strength (7403, 7410 and 7451) are characterized by having one or both of the elements from the group columbium and vanadium present in the base composition in combination with appreciable quantities of nitrogen and/or carbon.

It has been indicated herein that when either titanium or columbium, or both, is to be added to the alloy, a minimum of 0.25% be employed. Actually, smaller amounts of titanium and/or columbium could be present with some benefit, either as impurities or intentional additions, but their effectiveness would not be as significant as in the preferred range. When columbium is employed in the alloys, it will be understood that normal commercial sources of columbium, such as ferro-alloys thereof, may be used. Ordinarily, columbium so obtained will contain a small proportion of tantalum, and the final alloy may have tantalum present therein to this extent.

Many of the alloys in Table X were subjected to the RPI-type hot ductility test referred to earlier to determine their probable heat-affected zone behavior when subjected to the thermal cycles and stresses associated with welding. Most of the alloys had a rapid recovery of ductility when tested on cooling from the peak temperature, and would thus be expected to exhibit good weldability. Heat 7410 with the columbium addition and no molybdenum was marginal in this test.

As examples of the electrode and base metal welding characteristics of the basic Fe-Cr-Ni-Mn-Mo alloys of this invention a number of laboratory and production

welds were made with covered electrodes in both wrought and cast base metal. Typical welding conditions are given in Table XI and the compositions of the deposits are listed in Table XII. In spite of the fact that all the weld deposits were fully austenitic (i.e., no delta ferrite), no fissures were observed at 30 times magnification on the polished surfaces of side-bend specimens after bending, either in the weld bead or the heat-affected zone of the base metal. Satisfactory MIG welds have also been made using  $\frac{1}{16}$ " diameter bare wire with argon containing about 1% oxygen or pure argon in conjunction with a thin cathode stabilizing film on the wire.

STRESS-RUPTURE TESTS OF WELDS 170 AND 179 AT 1200° F.  
ALL WELD METAL SPECIMEN AS DEPOSITED. GAGE  
DIAMETER 0.505", LENGTH 3"

| 5  | Stress,<br>p.s.i. | Rupture<br>Time, hours | Rupture<br>Strain,<br>Percent | Reduction<br>of Area,<br>Percent | Minimum<br>Creep Rate,<br>Percent per<br>hour |
|----|-------------------|------------------------|-------------------------------|----------------------------------|-----------------------------------------------|
|    | 30,000            | 52                     | 13.8                          | 30.7                             | 0.10                                          |
|    | 25,000            | 178                    | 21.6                          | 34.2                             | 0.0087                                        |
| 10 | 20,000            | 832                    | 5.5                           | 21.0                             | 0.00062                                       |
|    | 17,500            | 1,963                  | 1.6                           | 11.8                             | 0.00021                                       |

Table XI

TYPICAL CONDITIONS USED IN WELDING THE ALLOYS OF THIS INVENTION

| Process            | Remarks                                                                                                    | Wire<br>Dia., in.                | Current,<br>amps   | Volts          | D.C.<br>Polarity      | Atmosphere  | Travel<br>Speed,<br>Inches/<br>min. | Interpass<br>Temperature,<br>°F. |
|--------------------|------------------------------------------------------------------------------------------------------------|----------------------------------|--------------------|----------------|-----------------------|-------------|-------------------------------------|----------------------------------|
| Covered Electrodes | Both titania and lime type coatings. Some alloying elements frequently added to coating.                   | $\frac{1}{16}$<br>$\frac{5}{32}$ | 100-120<br>145-160 | 24.5<br>22-27  | Reverse<br>do         |             |                                     | 200-300.                         |
| MIG                | Bare wire. Surface treated for cathode stabilization.                                                      | $\frac{3}{16}$                   | 180                | 22             | do                    |             |                                     | 200-300.                         |
| TIG                | $\frac{1}{4}$ " diameter tapered tungsten electrode. $\frac{5}{32}$ " diameter filler wire laid in groove. | $\frac{1}{16}$<br>$\frac{5}{32}$ | 280-320<br>280-320 | 24-28<br>24-28 | M-1<br>Straight<br>do | Argon<br>do | 12<br>12<br>6                       | 200-300.                         |
| TIG                | $\frac{3}{32}$ " diameter tungsten electrode. Butt weld between $\frac{1}{4}$ " thick plates.              | None                             | 80-90              | 11.5           | do                    | Helium      | 4                                   | Welded in one pass.              |

<sup>1</sup> Argon plus about 1% oxygen.

Table XII

COMPOSITIONS IN WEIGHT PERCENT<sup>1</sup> OF FULLY AUSTENITIC WELD DEPOSITS OF HIGHLY WELDABLE STAINLESS STEEL

| Weld No. | Cr   | Ni   | Mn   | Si  | Mo   | C    | N    | P    | S    |
|----------|------|------|------|-----|------|------|------|------|------|
| 167      | 17.9 | 16.4 | 7.61 | .48 | 2.77 | .045 | .048 |      |      |
| 170, 179 | 15.1 | 16.3 | 10.3 | .36 | 2.90 | .041 | .038 |      |      |
| 180      | 15.4 | 15.0 | 9.32 | .40 | 3.19 | .047 | .052 |      |      |
| 171      | 15.0 | 15.0 | 9.94 | .32 | 3.26 | .040 | .049 |      |      |
| 178      | 16.6 | 17.3 | 10.7 | .38 | 3.35 | .044 | .044 |      |      |
| 200      | 16.7 | 19.5 | 8.60 | .37 | 2.46 | .037 | .067 |      |      |
| S.P.     | 16.1 | 15.4 | 10.0 | .40 | 2.68 | .041 | .067 | .018 | .012 |

<sup>1</sup> Balance iron plus impurities.

The tensile properties of two of these welds are given in Table XIII at room temperature and elevated temperatures up to 2200° F., in both the as-deposited and solution treated conditions.

Table XIII

TENSILE PROPERTIES OF TITANIA TYPE COVERED ELECTRODE WELD DEPOSITS NO. 167 AND 170 XMN2054 CORE WIRE  $\frac{5}{32}$ " DIAMETER

| Condition                                               | Test<br>Temp.,<br>°F.                           | 0.2% Yield<br>Strength,<br>p.s.i.                       | Ultimate<br>Strength,<br>p.s.i.                        | Total<br>Elonga-<br>tion,<br>Percent         | Reduction<br>of<br>Area,<br>Percent          |
|---------------------------------------------------------|-------------------------------------------------|---------------------------------------------------------|--------------------------------------------------------|----------------------------------------------|----------------------------------------------|
| As Welded                                               | RT<br>1,100<br>1,350<br>1,600<br>1,900<br>2,200 | 56,000<br>31,600<br>27,200<br>18,500<br>8,900<br>4,000  | 77,600<br>52,300<br>36,600<br>19,900<br>9,200<br>4,200 | 42.2<br>36.7<br>53.3<br>50.3<br>19.0<br>27.3 | 61.2<br>60.8<br>54.7<br>50.8<br>24.8<br>35.0 |
| Solution Treated 1 hr. at 2,000° F. and water quenched. | RT<br>1,100<br>1,350<br>1,600<br>1,900<br>2,200 | 33,600<br>17,600<br>17,000<br>34,300<br>19,400<br>2,900 | 72,300<br>50,600<br>46.1<br>61.9<br>76.9<br>4,000      | 54.6<br>72.1<br>62.9<br>68.5<br>69.1<br>31.8 | 72.1<br>62.9<br>69.1<br>46.9<br>46.9<br>33.3 |

The soundness of the weld deposit was further demonstrated by the absence of microfissures on the surface of the room-temperature tensile specimen after test. It will be noted that there is a considerable decrease in strength up to 1350° F. with only a minor increase in ductility as a result of solution treatment, so that I usually prefer to use these welds in the as-deposited condition. The relatively good stress-rupture properties of typical weld metal deposits of highly weldable alloys made in accordance with this invention are set forth in Table XIV.

silicon, .04% carbon and the balance essentially iron. This alloy has low thermal conductivity at cryogenic temperatures, is dimensionally stable and has reasonably good strength without requiring work hardening or heat treatment. The alloy therefore has properties which make it useful for vessels, pipes, valves and Dewar flasks for containing liquefied gases. The low temperature properties of an alloy of this invention having the nominal composition set forth above are presented in Table XV. This alloy had a nitrogen content of approximately 0.04%

due to pick up during melting. Additions of nitrogen of up to 0.35% may be made to increase the strength of this alloy composition as well as other alloy compositions of this invention.

low temperature austenite stability and oxidation resistance must usually be considered.

During the course of my investigations, in which the above effects were fully considered, I discovered that

Table XV  
LOW TEMPERATURE PROPERTIES OF WELDABLE STAINLESS STEELS

| Test Temperature                                 | 70° F.              | -160° F. | -320° F.             | -423° F.             | -423° F.<br>Notched Bar<br>Kt=10 |
|--------------------------------------------------|---------------------|----------|----------------------|----------------------|----------------------------------|
| Cast Material Heat Treated, 1 Hr. 2,000° F.:     |                     |          |                      |                      |                                  |
| Tensile, p.s.i.                                  | 69,000              |          | 123,000              | 128,000              | 175,000                          |
| 2% Yield, p.s.i.                                 | 33,000              |          | 67,000               | 81,200               |                                  |
| .01% Yield                                       | 18,000              |          | 62,000               | 74,000               | 148,000                          |
| Elong., Percent                                  | 50                  |          | 66                   | 42.4                 |                                  |
| R.A., Percent                                    |                     |          | 49                   | 29.8                 | 23.8                             |
| Charpy Keyhole Impact, Ft. Lb.                   | 129                 | 82       | 88                   |                      |                                  |
| Weld Deposit Heat Treated, None:                 |                     |          |                      |                      |                                  |
| Tensile, p.s.i.                                  | <sup>a</sup> 77,000 |          | <sup>b</sup> 135,000 | <sup>c</sup> 163,000 | 220,600                          |
| 2% Yield, p.s.i.                                 | 57,000              |          | 102,000              | 122,000              |                                  |
| .01% Yield                                       | 49,000              |          | 97,000               | 115,000              | 200,000                          |
| Elong., Percent                                  | 42                  |          | 19                   | 17.0                 |                                  |
| R.A., Percent                                    | 61                  |          | 31                   | 26.7                 | 13.4                             |
| Charpy Keyhole Impact, Ft. Lb.                   | 47.5                |          | 31                   |                      |                                  |
| Wrought Material Heat Treated, 1 Hr., 2,000° F.: |                     |          |                      |                      |                                  |
| Tensile, p.s.i.                                  | 76,000              |          |                      |                      |                                  |
| 2% Yield, p.s.i.                                 | 32,000              |          |                      |                      |                                  |
| Elong., Percent                                  | 61                  |          |                      |                      |                                  |
| R.A., Percent                                    | 78                  |          |                      |                      |                                  |
| Charpy Keyhole Impact, Ft. Lb.                   | 148                 | 111      | 80                   |                      |                                  |

<sup>a</sup> All weld metal specimen.

<sup>b</sup> Transverse test, broke in weld.

<sup>c</sup> Transverse test, broke in heat-affected zone of wrought base metal.

### HIGH STRENGTH WELDABLE STAINLESS STEELS

The alloys described above, particularly those of Tables IV and X and similar alloys, have been found to be highly satisfactory for many purposes requiring reasonably strong, highly weldable stainless steels. There are, however, many applications requiring stainless steels having greater strength than the alloys described previously. For such applications, the highly crack resistant alloy compositions described above are modified at some sacrifice in weldability to assure the required additional strength as described hereafter. In modifying these compositions the principles set forth previously are carefully followed so as to achieve optimum properties for the intended application.

Ordinarily, increased strength would be secured by increasing the proportions of the principal alloying strengtheners, i.e., molybdenum, carbon and nitrogen, or by additions of tungsten, vanadium or columbium. The limits within which these constituents may be increased or added to the alloys are defined by the requirement that the high degree of weldability achieved by proper balance of the Fe-Cr-Ni-Mn-Mo base constituents, in accordance with this invention, be retained as much as possible. Thus, the optimum combination of manganese and molybdenum for rupture strength and resistance to hot-cracking in welding or casting has been described above and in FIG. 5, and to deviate significantly from this optimum ratio, will inevitably have a detrimental effect on these properties. In addition to the hot-cracking tendencies, the effects of alloying elements on one or more of the following factors, such as, delta ferrite formation, sigma precipitation, stress-rupture ductility,

combinations of one or more of the elements from the group boron, zirconium and vanadium taken in combination with nitrogen produced alloys of exceptionally high strength while still retaining excellent weldability, as will be evident from the following examples and description.

The effects of boron, zirconium and vanadium in addition to nitrogen were investigated singly and in various combinations with the results given in Table XVI. From 45 results on heat 7441 (Table X) with 3.2% V, it would have been anticipated that 0.57% V would have had a negligible effect in heat 7471, but unexpectedly, the vanadium and nitrogen interacted and produced a strength well beyond the sum of the effects of the individual elements. Similarly, boron plus nitrogen (heats 50 7467, 7478) and zirconium plus nitrogen (heat 7480) had individual strengthening effects, but the combination of boron, zirconium and nitrogen produced unexpectedly high strength and excellent ductility in the 55 alloy of heat 7479. It is apparent that steels having excellent properties which exceed those of commercially produced stainless steels can be obtained by employing one or more of the elements from the group consisting of boron, zirconium and vanadium taken in conjunction 60 with high nitrogen in the crack resistant alloy base. From these and other tests the useful ranges of these elements have been determined to be 0.002% to 0.03% boron, 0.002% to 0.06% zirconium, 0.15% to 1% vanadium, and 0.10% to 0.35% nitrogen. It is the unique combination 65 of manganese and molybdenum, in the alloys of this invention, that enables me to obtain a high degree of weldability in these high strength alloys, in spite of the presence of boron and zirconium, which in FIG. 3 are shown to be detrimental in the simple iron-chromium-nickel alloys insofar as hot-cracking is concerned.

Table XVI

SUMMARY OF 1200° F. STRESS-RUPTURE AND CREEP PROPERTIES OF WELDABLE STAINLESS STEELS WITH ADDITIONS OF BORON, ZIRCONIUM, VANADIUM AND NITROGEN

| Heat No. | Weight Percent |        |       |      | 1,000 Hour Properties  |                         | Stress for 0.01% per hour Minimum Creep Rate, p.s.i. |
|----------|----------------|--------|-------|------|------------------------|-------------------------|------------------------------------------------------|
|          | N              | B      | Zr    | V    | Rupture Stress, p.s.i. | Rupture Strain, Percent |                                                      |
| 7470     | .13            |        |       |      | 23,000                 | 20                      | 22,000                                               |
| 7471     | .11            |        |       |      | 25,000                 | 7                       | 32,000                                               |
| 7457     | .11            | .0037  |       |      | 26,500                 | 60                      | 22,000                                               |
| 7478     | .091           | .006   |       |      | 26,500                 | 50                      | 26,000                                               |
| 7480     | .12            | .0019  | .0098 |      | 25,000                 | 34                      | 22,500                                               |
| 7479     | .12            | .0045  | .003  |      | 33,000                 | 30                      | 32,000                                               |
| 7489     | .12            | .0051  | .017  |      | 34,000                 | 40                      | 40,000                                               |
| 7488     | .13            | (.005) | .0086 | (.3) | 35,000                 | 27                      | 38,000                                               |

<sup>1</sup> Residual boron from impurities in the charge or crucible—No intentional addition.  
( )=aim composition.

The preferred alloy composition adds to the previously defined Fe-Cr-Ni-Mo-Mn alloy base the beneficial strengthening effects of all of the elements of the group boron, zirconium and vanadium in conjunction with nitrogen. The marked improvements in rupture and creep strength produced by the combined addition of B, Zr and V at a given N level are shown in FIGS. 10 and 11. Curve A in each case was obtained in testing an Fe-Cr-Ni-Mo-Mn alloy base containing nitrogen. Curve B was obtained in testing the alloy base with additions of B, Zr, V and N. Not only are the curves raised by the combination of these addition elements, but the increased slope in the initial portion of each curve B indicates a synergistic interaction between (B, Zr, V) and N. These elements within the preferred composition range, by a mechanism not fully understood, produce a steel of unusually high strength and ductility. This unique alloy containing boron, zirconium, vanadium and nitrogen is an extremely desirable high-strength stainless steel which is more weldable than some of the commercially available stainless steels having even lower strength.

A high strength stainless steel alloy in which the alloy constituents are balanced to provide the desired high level of strength without forming undue amounts of sigma with its consequent embrittling effect, comprises, from 14% to 16% chromium, from 20% to 24% nickel, from 8% to 13% manganese, from 1.5% to 3% molybdenum, the total of manganese and molybdenum being from 11% to 16%; from 0.15% to 0.35% vanadium, from 0.003% to 0.02% boron, from 0.003% to 0.04% zirconium, from 0.02% to 0.06% carbon, from 0.2% to 0.25% nitrogen, up to 4% silicon, and the balance essentially iron and small amounts of incidental impurities.

Another preferred range of composition of the high strength weldable stainless steel alloy is 15-17% Cr, 18.5-22% Ni, about 8-13% Mn, 1.5-3.0% Mo, the total of manganese and molybdenum being from 11% to 16%, 0.15-0.35% V, 0.004-0.02% B, 0.005 to 0.04% Zr, 0.10 to 0.25% N, 0.01 to 0.06% C, up to 0.4% Si and balance iron and incidental impurities. A particularly useful high strength alloy for steam turbine piping applications contains about 16% Cr, about 20% Ni, about 11% Mn, about 2.25% Mo, about 0.25% V, about 0.006% B, about 0.015% Zr, about 0.04% C, about 0.20% N, less than about 0.25% Si, and the balance iron and small amounts of incidental impurities.

Even higher strengths can be provided by employing quantities of boron and zirconium exceeding the preferred ranges above specified, but for applications involving diffi-

cult welding or casting operations, boron and zirconium should be kept at the specified low levels to avoid hot-cracking of weld deposits, heat-affected zone cracking of base metal during welding and hot-tearing of castings as previously explained.

The powerful effect of nitrogen on rupture and creep strength of steels containing B, Zr and V is shown by curve B in FIGS. 10 and 11, as mentioned previously, and the data in Tables XVI and XVII. Rupture strength approaches a maximum at about 0.2% nitrogen. The corresponding 1000 hour stress-rupture elongation at 1200° F. drops rapidly from about 80% to 40% between 0.02% and 0.04% N, as illustrated in FIG. 12, but decreases very slowly at higher nitrogen contents up to 0.13% and higher. Thus, at the high strength level corresponding to 0.19% to 0.23% nitrogen, the elongation is greater than 30%. In general, stress rupture elongation is a minimum in tests lasting about 100 to 300 hours. In tests lasting about 1000 hours and longer, the ductility increases again, contrary to general experience in stainless steel, as illustrated by the typical stress-rupture tests results set forth in Table XVII.

Table XVII

STRESS-RUPTURE PROPERTIES OF HIGH STRENGTH WELDABLE STAINLESS STEEL HEAT 7489 FORGED  $\frac{1}{8}$ " DIAMETER BAR SOLUTION TREATED 1 HOUR AT 1000° F.

| Test Temp., °F. | Stress, p.s.i. | Rupture Time, hours | Rupture Strain, percent | Reduction of Area, percent | Minimum Creep Rate, percent per hour |
|-----------------|----------------|---------------------|-------------------------|----------------------------|--------------------------------------|
| 1,100           | 40,000         | 9538+               | 9.9+                    |                            | 0.00013                              |
| 1,200           | 50,000         | 20                  | 18.9                    | 20.0                       | 0.19                                 |
|                 | 45,000         | 84                  | 15.6                    | 37.3                       | 0.040                                |
|                 | 40,000         | 349                 | 18.4                    | 25.2                       | 0.0071                               |
|                 | 35,000         | 869                 | 39.3                    | 61.6                       | 0.0035                               |
| 11,350          | 20,000         | 188                 | 61.9                    | 79.2                       | 0.040                                |
| 1,500           | 10,000         | 145                 | 70.3                    | 84.0                       | 0.081                                |

<sup>1</sup> Test on heat 7488.

The 1200° F. stress-rupture and creep properties of heat 7489 in the above table may be compared with the similar properties of other high strength weldable stainless steels of this invention and with those of the highly weldable stainless steels of this invention in Tables IV, X, XVI and XVIII where the 1000 hour properties are summarized. The tensile and yield strengths of the high strength weldable steels both at room temperature and at 1025° F. increase markedly and in an approximately linear fashion with increase in nitrogen as shown in FIG. 13.

27  
Table XVIII

SUMMARY OF 1200° F. STRESS-RUPTURE AND CREEP STRENGTHS OF HIGH STRENGTH WELDABLE STAINLESS STEELS

| Heat No. | 1,000 Hour Properties  |                         | Stress for 0.01% per hour Minimum Creep Rate, p.s.i. |
|----------|------------------------|-------------------------|------------------------------------------------------|
|          | Rupture Stress, p.s.i. | Rupture Strain, percent |                                                      |
| 7486     | 35,000                 | 22                      | 40,000                                               |
| 7530     | 21,000                 | 55                      | 22,000                                               |
| 7531     | 26,000                 | 10                      | 28,000                                               |
| 7532     | 28,000                 | 30                      | 30,000                                               |
| 7533     | 27,000                 | 20                      | 30,000                                               |
| 7534     | 30,000                 | 21                      | 33,000                                               |
| 7535     | 25,000                 | 45                      | 25,000                                               |
| 7571     | 35,000                 | 30                      | 39,000                                               |
| 7572     | 34,000                 | 34                      | 42,500                                               |
| 7577     | 36,000                 | 26                      | 39,000                                               |
| VM545    | 38,000                 | 40                      | 43,000                                               |
| XMM2232  | 30,500                 | 13                      | 37,000                                               |
| XMM2239  | 27,000                 | 22                      | 29,500                                               |
| XMM2240  | 28,500                 | 20                      | 34,000                                               |
| XMM2265  | 31,000                 | 40                      | 35,000                                               |
| KV101    | 34,000                 | 35                      | 41,000                                               |

It is a further characteristic of these high strength stainless steels that stresses higher than 62.5% of the yield strength and higher than 25% of the tensile strength can be applied without exceeding the boiler code stresses for minimum creep rate or stress-rupture life. For a fuller utilization of the high temperature capabilities of these alloys, it is, therefore, desirable to find ways of increasing the short-time yield and tensile strengths. For service temperatures up to about 1200° F., I have found that a fine austenite grain size produced by adequate prior hot or cold working and a low temperature solution heat treatment in the range of about 1650 to 1800° F. will increase the yield strength of wrought material to equal or even exceed that of argon shielded weld deposits or of the weld joint in tungsten inert gas welded plates.

Adequate prior hot working in these fully austenitic materials is achieved by control of initial soaking temperature, and holding time, amount of the reduction, finishing temperature, and reheating schedule. Preferably, the initial working temperature should only be high enough to provide ease of deformation and the finishing temperature should be low enough so that some "hot-cold" working occurs. Under these conditions the steel can be fully recrystallized to a uniform grain size finer than ASTM No. 6 by solution treatments for one hour at temperatures in the range of about 1650° F. to 1900° F. When the steel is solution treated below about 1775° F., particles of an undissolved precipitate contribute to the yield and tensile strength. Tensile properties of hot-rolled and solution treated plate made from the high strength stainless steel of this invention are set forth in Table XIX.

Table XIX

TENSILE PROPERTIES OF COMMERCIALLY HOT-ROLLED  $\frac{1}{4}$ " PLATE OF HIGH STRENGTH WELDABLE STEEL HEAT XMM2265

| Heat Treatment |            |       |            | Test Temp., °F. | 0.2% Yield Strength, p.s.i. | Ultimate Strength, p.s.i. | Elongation in 2", percent | Reduction of Area, percent |
|----------------|------------|-------|------------|-----------------|-----------------------------|---------------------------|---------------------------|----------------------------|
| Hours          | Temp., °F. | Hours | Temp., °F. |                 |                             |                           |                           |                            |
| 1              | 1,850      |       |            | RT              | 44,000                      | 102,000                   | 43                        | 48                         |
| 1              | 1,800      |       |            | RT              | 45,000                      | 102,000                   | 43                        | 50                         |
| 1              | 1,750      |       |            | RT              | 48,000                      | 104,000                   | 42                        | 51                         |
| 1              | 1,700      |       |            | RT              | 50,000                      | 105,000                   | 37                        | 48                         |
| 20             | 1,350      | 1     | 1,700      | 1,025           | 37,000                      | 82,000                    | 32                        | 47                         |
| 20             | 1,500      | 1     | 1,700      | 1,025           | 35,000                      | 82,000                    | 34                        | 44                         |
| 1              | 1,700      |       |            | 1,025           | 33,000                      | 82,000                    | 35                        | 51                         |
| 1              | 1,850      |       |            | 1,025           | 31,000                      | 81,000                    | 35                        | 48                         |
| 1              | 1,900      |       |            | 1,025           | 27,000                      | 78,000                    | 44                        | 50                         |

For additional strengthening or in articles such as large forgings where it is difficult to introduce uniform work hardening, a heat treatment for about 20 hours in the range of about 1300° F. to 1550° F. will precipitate substantial amounts of a second phase as dispersed particles,

28

probably the sigma phase. Upon subsequent solution treatment for one hour at temperatures between about 1650° F. and 1800° F., the matrix recrystallizes and a part of the precipitate remains as small spheroidized particles dispersed throughout the grains. These particles provide barriers to slip and account for the higher yield strengths at 1025° F. of the samples aged at 1350° F. and 1500° F. prior to the 1700° F. solution treatment (see Table XIX). However, this precipitation prior to testing has little effect on the long time creep or rupture properties because aging occurs at elevated temperatures in service in any event.

The tensile properties of a high strength austenitic stainless steel of this invention, containing boron, zirconium, vanadium and a high nitrogen content of 0.23% were determined over a wide range of temperatures extending as low as -320° F. and as high as 2000° F. (see Table XX). The strength and ductility of this alloy at cryogenic temperatures (-320° F.) was quite remarkable. Since the boron and zirconium make little or no contribution to strength or ductility at such low temperatures, alloys containing only nitrogen, in addition to the basic iron-chromium-nickel-manganese-molybdenum alloy (with or without vanadium), will display essentially the same good low temperature tensile properties as the alloy of Table XX. The object of using an alloy without the boron and zirconium addition for cryogenic applications would be to secure better weldability.

Table XX

TENSILE PROPERTIES OF HIGH STRENGTH STAINLESS STEEL HEAT 7572 $\frac{1}{2}$ " DIAMETER FORGED BARS SOLUTION TREATED 1 HOUR AT 1700° F.

| Test Temp. °F. | 0.2% Yield Strength, p.s.i. | Ultimate Strength, p.s.i. | Total Elongation, Percent | Reduction of Area, Percent |
|----------------|-----------------------------|---------------------------|---------------------------|----------------------------|
| -320           | 135,500                     | 200,000                   | 57.0                      | 53.5                       |
| RT             | 84,400                      | 116,200                   | 33.1                      | 55.0                       |
| 1,025          | 53,600                      | 82,000                    | 26.5                      | 57.3                       |
| 1,350          | 48,800                      | 61,100                    | 24.8                      | 59.2                       |
| 1,600          | 35,300                      | 37,500                    | 38.9                      | 49.6                       |
| 2,000          | 9,500                       | 9,700                     | 26.8                      | 30.3                       |

In structural and pressure vessel design it is usually preferred that the yield strength of the weld metal be greater than that of the base metal to avoid strain concentration in the event of overstressing. I therefore prefer to select a solution temperature for the base material prior to welding high enough to give a yield strength slightly lower than that of the type weld deposit to be used. I prefer not to solution treat the welded joints because this results in a substantial reduction in their yield and tensile strength. The high strength of as deposited weld metal is obtained in spite of a coarse grain size and may be due to such effects as the cellular structure with-

in the grains, segregation during freezing or lattice imperfections resulting from the solidification process. A solution treatment seems to markedly reduce such strengthening mechanisms. In the absence of substantial amounts of hot or cold working, which are impractical to apply

to most welded structures, it has also been found that aging of the weld deposit before solution treatment is ineffective in maintaining the original strength.

Some tensile properties of several high strength weld metals are given in Table XXI. The conditions employed in making the welds are summarized in Table XI and the compositions of these and other deposits are listed in Table XXII. To some extent for most elements,

stronger than the weld number 230. The tensile properties of a TIG weld with filler wire were comparable to those of the covered electrode deposit. When fittings and pipe are fabricated from plate by tungsten inert gas seam welding, with or without filler wire the base metal yield strength should be adjusted to be just below the appropriate weld strength, by suitable heat treatment of the plate prior to welding.

Table XXI  
TENSILE PROPERTIES OF SOME HIGH STRENGTH STAINLESS STEEL WELDS AS DEPOSITED

| Electrode<br>Wire Heat<br>No. | Weld<br>No. | Process                                                                                                  | Test<br>Temp.,<br>°F. | 0.2% Yield<br>Strength,<br>p.s.i. | Ultimate<br>Strength,<br>p.s.i. | Total<br>Elongation,<br>Percent | Reduction<br>of Area,<br>Percent |
|-------------------------------|-------------|----------------------------------------------------------------------------------------------------------|-----------------------|-----------------------------------|---------------------------------|---------------------------------|----------------------------------|
| 7487                          | 230         | Argon Shielding. MIG $\frac{1}{16}$ " dia. wire Cathode stabilized.                                      | RT<br>1,025           | 51,300<br>29,500                  | 87,600<br>59,500                | 46.6<br>39.2                    | 64.9<br>60.1                     |
| XMM2232                       | 432A        | Covered Electrode Lot 3A $\frac{5}{32}$ " dia. wire.                                                     | RT<br>1,025           | 62,100<br>38,800                  | 94,000<br>64,500                | 44.5<br>41.5                    | 61.2<br>62.6                     |
| XMM2277                       | 484B        | TIG. Argon shielding $\frac{5}{32}$ " dia. filler wire.                                                  | RT<br>1,025           | 64,100<br>40,400                  | 93,900<br>64,400                | 30.5<br>26.0                    | 44.3<br>34.3                     |
| None                          | T.T.        | TIG. Helium shielding Butt joint between two $\frac{3}{4}$ " plates. No filler wire. XMM2265 base metal. | RT<br>1,025           | 53,000<br>32,000                  | 96,000<br>69,000                | 25.0<br>18.5                    | 62.5<br>55.5                     |

NOTE.—Transverse flat sheet tensile specimen fractured in the weld.

Table XXII  
COMPOSITIONS OF HIGH STRENGTH STAINLESS STEEL WELD DEPOSITS IN WEIGHT PERCENT  
(BALANCE IRON PLUS IMPURITIES)

| Core Wire Heat<br>No. | Weld No. | Type Weld   | Cr   | Ni   | Mn   | Si    | C     | N   | Mo   | V     | B     | Zr     |
|-----------------------|----------|-------------|------|------|------|-------|-------|-----|------|-------|-------|--------|
| 7487                  | 230      | MIG         | 16.5 | 20.7 | 11.5 | .12   | .035  | .12 | 2.09 | .28   | .0038 | .004   |
| XMM2265               | 398      | MIG         | 15.0 | 20.1 | 12.2 | .41   | .022  | .14 | 2.24 | .26   | .014  | .028   |
| XMM2232               | 58-1     | C.E. Lot 1  | 16.0 | 19.5 | 8.29 | .82   | .048  | .14 | 2.25 | .33   | .0053 | .0016  |
| XMM2232               | 370      | C.E. Lot 2  | 14.8 | 19.1 | 12.3 | 1.08  | .046  | .12 | 2.04 | .30   | .0043 | .0019  |
|                       | 432      |             |      |      |      |       |       |     |      |       |       |        |
| XMM2232               | 451      | C.E. Lot 3  | 16.0 | 20.3 | 10.4 | .57   | .051  | .16 | 2.52 | .29   | .0074 | .006   |
| XMM2232               | 452A     | C.E. Lot 3A | 16.1 | 20.3 | 10.3 | .52   | .048  | .18 | 2.50 | .30   | .0067 | <.004  |
| XMM2277               | 523      | C.E. Lot 4  | 16.8 | 21.3 | 10.9 | .43   | .024  | .19 | 2.31 | .26   | .012  | <.0025 |
| XMM2232               | 460      | TIG         | (16) | (20) | 8.96 | (.37) | (.03) | .12 | 2.16 | (.25) | .012  | .0055  |
| XMM2277               | 484B     | TIG         | 16.0 | 20.5 | 11.7 | .19   | .013  | .14 | 2.32 | .30   | .023  | .038   |
| VM545                 | 484C     | TIG         | 16.6 | 20.1 | 12.2 | .05   | .012  | .17 | 2.40 | .27   | .014  | .0095  |

C.E.=covered electrode. Supplementary metal additions made in all these coatings.  
(Parentheses indicate nominal composition.)

but particularly in the case of reactive elements such as B and Zr, compensation must be made in the core wire or coating for losses during transfer across the arc. Considerable excesses of B and Zr are needed for covered electrodes. The covered electrode deposit weld number 432A of Table XXI has substantially higher strength than the argon shielded consumable metal weld number 230. The tungsten arc, helium shielded butt weld joint in a  $\frac{1}{4}$ " thick plate of heat XMM2265 is somewhat

45

When it comes to stress-rupture and creep strength, the situation is partially reversed. As shown in Table XXIII, the covered electrode deposits are considerably weaker, probably because of partial loss or oxidation of boron and zirconium by the atmosphere and slag coating. The TIG welds made with filler metal have especially excellent properties. The TIG weld made with the vacuum melted filler wire (heat VM 545) is particularly noteworthy because of the high stress-rupture ductility.

Table XXIII  
STRESS-RUPTURE PROPERTIES AT 1200° F. OF SOME HIGH STRENGTH STAINLESS STEEL WELDS—AS DEPOSITED

| Electrode<br>Heat No. | Process                                                | Weld No.   | Stress,<br>p.s.i.                                                                                                              | Rupture<br>Time,<br>hours                                    | Percent<br>Rupture<br>Strain                                                                          | Percent<br>Reduction<br>of Area                                                                                                         | Minimum<br>Creep Rate,<br>Percent per<br>hour.                                                                           |
|-----------------------|--------------------------------------------------------|------------|--------------------------------------------------------------------------------------------------------------------------------|--------------------------------------------------------------|-------------------------------------------------------------------------------------------------------|-----------------------------------------------------------------------------------------------------------------------------------------|--------------------------------------------------------------------------------------------------------------------------|
| 7487                  | MIG                                                    | 230        | 40,000<br>35,000<br>30,000<br>25,000                                                                                           | 24<br>74<br>2,016<br>8,990+                                  | 12.0<br>10.0<br>7.3<br>7.1+                                                                           | 24.9<br>23.2<br>19.6<br>14.5                                                                                                            | 0.014<br>0.0052<br>0.00045<br>0.00015                                                                                    |
| XMM2232               | Covered Electrode Lot 3A                               | 432A, 451A | 40,000<br>35,000<br>30,000<br>25,000<br>40,000<br>35,000<br>30,000<br>25,000<br>35,000<br>30,000<br>45,000<br>40,000<br>35,000 | 29<br>58<br>164<br>1,553<br>224<br>751<br>129<br>536<br>670+ | 3.3<br>1.3<br>1.0<br>1.0<br>17.6<br>10.4<br>11.3<br>5.3<br>30.1<br>4.7<br>27.5<br>4.0<br>16.7<br>18.6 | 14.5<br>16.2<br>5.4<br>4.7<br>27.5<br>4.0<br>16.7<br>18.6<br>59.3<br>0.031<br>0.0054<br>0.00062<br>0.00025<br>0.011<br>0.0046<br>0.0011 | 0.011<br>0.0054<br>0.00062<br>0.00025<br>0.031<br>0.011<br>0.0046<br>0.0011<br>0.23<br>0.17<br>0.17<br>0.0008<br>0.00025 |
| None                  | TIG. Butt joint in $\frac{3}{4}$ " plates of XMM 2265. |            |                                                                                                                                |                                                              |                                                                                                       |                                                                                                                                         |                                                                                                                          |
| XMM2277               | TIG. $\frac{5}{32}$ " rods fused in groove.            | 484B       | 45,000<br>40,000<br>35,000                                                                                                     | 49<br>574<br>992<br>665+                                     | 30.1<br>22.7<br>19.3                                                                                  | 59.3<br>42.0<br>45.0                                                                                                                    | 0.23<br>0.17<br>0.0008                                                                                                   |
| VM545                 | TIG. $\frac{5}{32}$ " rods fused in groove.            | 484C       | 50,000<br>45,000<br>40,000<br>35,000                                                                                           | 49<br>574<br>992<br>665+                                     | 30.1<br>22.7<br>19.3                                                                                  | 59.3<br>42.0<br>45.0                                                                                                                    | 0.23<br>0.17<br>0.0008                                                                                                   |

In the preparation of certain covered electrodes of high-strength weldable stainless steel, a high silicon ferro-zirconium was added to the coating to compensate for zirconium losses during welding. As a result, the silicon contents of these deposits were 0.82 and 1.08% (see Table XXII). Side bends of these welds all showed a small amount of fissuring. For certain covered electrodes a nickel-zirconium powder was used instead, and the silicon contents of the deposits were 0.52 and 0.57%. Neither of these welds showed any fissures in five side bends. An increase in silicon in these weld deposits of about 0.2% over that present in the core wire comes from reaction of the molten metal with the electrode coating ingredients. For the reasons noted above, in order to keep the silicon content below about 0.6% in covered electrode deposits of the high strength alloys of this invention, I prefer to have less than about 0.4% silicon in the core wire for covered electrodes.

In the case of MIG welding (consumable metal inert gas arc welding), the silicon content seems to be even more critical than for covered electrode welding. A MIG weld deposit containing 0.41% silicon was badly fissured in a highly restrained weld, whereas another deposit with 0.12% silicon showed only an occasional fissure under similar conditions. For the wire for MIG welding of high strength steels I therefore prefer to keep the silicon content below about 0.25%.

It is also a characteristic of inert gas shielded welding that boron and zirconium are transferred more efficiently than in covered electrode welding. Hence the wire for MIG and TIG welding should contain lesser amounts of these elements than are required in the core wire of covered electrodes to minimize hot-cracking problems.

From such high strength austenitic stainless steel alloys large diameter welded tubing has been successfully made by commercial techniques in a section about 10 feet long. The tubing was formed from .280 inch thick sheet of heat XMM 2265 which was first shaped to cylindrical form. Tungsten inert gas welding (helium) was used with electrode tips on the top and bottom sides of the joint to make the seam weld, the bottom electrode leading the top electrode by 1 inch in melting. Welding was carried out at a rate of about 4 inches per minute. The irregularities were ground off and the weld-bead was rolled smooth or "planished." The tubing was then put through sizing rolls to control the concentricity and diameter. The final outside diameter of the tubing was 10.7 inches. In general, the high strength stainless steel worked in a manner similar to conventional stainless steel in this process. A welded 90° elbow of this size was made.

Melting practice for these high strength stainless steels follows current commercial air melting practices for austenitic stainless steels. The recovery of vanadium is fairly consistent, so that this element in suitable form may be added either late in the heat or in the ladle. However, boron and zirconium require particular care to avoid melting losses and erratic recoveries. Master alloys or ferro alloys of these elements will dissolve more readily and the additions will pass through the slag with smaller losses. Holding time in the furnace must be held to the minimum needed for adequate mixing to prevent reaction with the slag or refractories. Although ferrozirconium has been used successfully, this ferro alloy contains about 40% silicon. Nickel-zirconium and chromium-zirconium master alloys, or similar sources of zirconium may be used in order to help keep the silicon content below about 0.6% and preferably below about 0.25% in the alloy. Boron and zirconium are preferably added in the ladle. A small amount of a strong deoxidizer such as CaSi, aluminum or titanium may be added in the furnace prior to the boron or zirconium additions to improve the recoveries. Titanium in amounts of 0.05 and 0.10% was used in some heats for this purpose. Additions of boron to the

charge have been made in the range of 0.002 to 0.02% and of zirconium in the range of 0.005 to 0.15%. Analyses of bar stock from these heats show a range in boron from 0.002% to 0.025% and in zirconium from 0.003% to 0.06%.

Vacuum induction melting has also been employed in making the high strength alloys of this invention. In this process the iron, chromium, nickel and molybdenum are first melted under vacuum and then deoxidized with carbon and/or hydrogen. In order to prevent losses of manganese and nitrogen, a partial pressure of an inert gas or nitrogen is introduced in the furnace for the balance of the melting operation. After the manganese addition, nitrogen is added as Mn-N or a high nitrogen containing ferrochromium. Vanadium, boron and zirconium are added just before pouring. Because of the low oxygen content of these melts it is not necessary to add deoxidizers, such as CaSi or Ti. Moreover, the recoveries of Mn, N, B and Zr charged are considerably higher than in air melting. Wrought specimens made from a vacuum melted heat (VM545) have exhibited exceptionally high rupture strengths and ductilities, and a TIG weld (No. 484-C) made with VM545 filler wire had the highest strength of any weld or wrought specimen tested along with good rupture ductility and absence of microfissures in the weld made in a 1 1/8" grooved plate of heat XMM 2284. From the excellent properties of laboratory air melted heats with only 0.09% silicon and the vacuum melt with less than 0.02% silicon, I conclude that silicon is not an essential element of the alloy and in fact must be limited below certain maximum amounts to minimize hot-cracking. When silicon is employed as a deoxidizer, it will naturally be present in amounts of greater than about 0.08% up to a maximum of about 1%. For vacuum melting or if other deoxidation practice is used, there need be no lower limit on silicon.

For a few applications requiring added strength or corrosion resistance in the as welded condition and when the welding conditions are not especially severe, I add from 0.25 to 1.5% columbium and preferably from 0.5% to 1.0% columbium to these high strength steels. In order to maintain adequate weldability when B, Zr and Cb are all present, the composition of the alloy with respect to Mn, Mo, and maximum amounts of B and Zr is held within close limits. A preferred alloy containing columbium comprises by weight from 14% to 18% chromium, from 15% to 26% nickel, from 11% to 13% manganese, from 1% to 3% molybdenum, with manganese plus molybdenum from 12% to 15% total, from 0.5% to 1.0% columbium, from 0.002% to 0.015% boron, from 0.003% to 0.3% zirconium, from 0.15% to 0.35% V, from 0.01% to 0.06% carbon, from 0.10% to 0.25% nitrogen, up to 0.4% silicon and balance iron and incidental impurities, and in which alloy the composition function  $F(c)$  is greater than 14 and the function  $\phi(c)$  is from 1 to 3.75.

#### PRECIPITATION HARDENABLE, HIGH STRENGTH WELDABLE STAINLESS STEELS

In an earlier section of this specification it was shown (Table X) that titanium up to 1.15% had little effect on rupture strength in the steels of this invention. The principal effect on properties that has been noted is a marked increase in the tensile ductility at elevated temperatures. Improvement appears with even 0.14% titanium and continues or even increases up to 2% titanium and higher as shown in Table XXIV. A more detailed survey reported in Table XXV for heat number 7570 over the range of temperatures from -320° F. to 2000° F. shows the same effect. At 2000° F. some of the specimens neck down to a point as small as the end of a lead pencil, indicating an unusual capacity for hot working without fissuring that would be useful in commercial forming operations of the alloy.

Table XXIV

## EFFECT OF TITANIUM ON THE TENSILE STRENGTH AND DUCTILITY OF STAINLESS STEELS AT ELEVATED TEMPERATURES

| Heat No. | Percent Ti | Test Temp., °F. | 0.2% Yield Strength | Ultimate Strength, p.s.i. | Elongation, Percent | Reduction of Area, Percent |
|----------|------------|-----------------|---------------------|---------------------------|---------------------|----------------------------|
| 7431     | 0          | RT              | 28,100              | 77,600                    | 54.8                | 75.7                       |
|          |            | 1,350           | 12,800              | 37,200                    | 47.9                | 45.6                       |
|          |            | 2,000           | 5,500               | 6,200                     | 35.0                | 34.3                       |
| 7448     | 0.14       | RT              | 33,700              | 80,500                    | 59.1                | 72.7                       |
|          |            | 1,350           | 18,000              | 37,600                    | 65.1                | 67.2                       |
|          |            | 2,000           | 6,200               | 7,200                     | 98.3                | 77.2                       |
| 7458     | 0.41       | 1,350           | 13,700              | 35,800                    | 44.8                | 41.4                       |
|          |            | 2,000           | 5,400               | 6,500                     | 102.3               | 90.8                       |
|          |            | 2,000           | 5,400               | 6,500                     | 52.7                | 79.4                       |
| 7459     | 0.99       | RT              | 29,200              | 77,700                    | 47.6                | 44.7                       |
|          |            | 1,350           | 15,000              | 37,800                    | 88.4                | 97.4                       |
|          |            | 2,000           | 6,000               | 6,800                     | 56.6                | 78.9                       |
| 7411     | 1.15       | RT              | 29,700              | 77,200                    | 81.3                | 79.4                       |
|          |            | 1,350           | 13,800              | 35,700                    | 52.0                | 60.8                       |
|          |            | 2,000           | 4,600               | 5,200                     | 112.6               | 69.2                       |
| VM546    | 1.8        | RT              | 73,600              | 143,200                   | 41.3                | 99.5                       |
|          |            | 1,350           | 54,300              | 77,200                    | 174.9               |                            |
|          |            | 2,000           | 5,100               | 5,900                     |                     |                            |

Table XXV

## TENSILE PROPERTIES OF PRECIPITATION HARDENABLE, WELDABLE STAINLESS STEEL HEAT NO. 7570

| Test Temp., °F. | 0.2% Yield Strength, p.s.i. | Ultimate Strength, p.s.i. | Total Elongation, Percent | Reduction of Area, Percent |
|-----------------|-----------------------------|---------------------------|---------------------------|----------------------------|
| -320            | 113,400                     | 179,000                   | 35.6                      | 50.1                       |
| RT              | 100,700                     | 144,500                   | 28.1                      | 50.0                       |
| 1,025           | 79,700                      | 116,800                   | 20.1                      | 39.2                       |
| 1,350           | 55,700                      | 70,500                    | 25.0                      | 28.2                       |
| 1,600           | 17,800                      | 21,200                    | 58.4                      | 97.6                       |
| 2,000           | 5,100                       | 8,800                     | 107.4                     | 99.3                       |

There is a remarkable difference, however, between the yield strengths and tensile strengths of heats VM 546 and 7570 and those of the first group of five steels of Table XXIV whose strength properties are very similar. The difference is made possible by a precipitation hardening reaction during aging that becomes effective in reasonable time periods above about 1.5% titanium in this alloy base.

Age hardening with  $\text{Ni}_3\text{Ti}$  has been employed in many prior art iron-base alloys. In such alloys, however, the titanium content leads to very poor welding performance and weld deposits and heat-affected zones exhibit severe cracking in moderately restrained joints. In contrast to this behavior, I have discovered that within certain narrow ranges of my crack resistant alloy base, titanium can be added in amounts of 1.5% to 2.5% to obtain a substantial increase in hardness on aging and still retain satisfactory weldability. Compositions of three of these steels are shown in Table XXVI and the excellent rupture strengths are summarized in Table XXVII. For comparison, there is shown a heat (#7569) containing titanium in an amount below the critical range. This heat reached a moderately good strength level but only after prolonged aging.

Table XXVII

## SUMMARY OF 1200° F. STRESS-RUPTURE AND CREEP PROPERTIES OF PRECIPITATION HARDENABLE, WELDABLE STAINLESS STEEL

| Heat No. | Form    | 1000 Hour Properties   |                         | Stress for 0.01% per Hour Minimum Creep Rate, p.s.i. |
|----------|---------|------------------------|-------------------------|------------------------------------------------------|
|          |         | Rupture Stress, p.s.i. | Rupture Strain, Percent |                                                      |
| 7569     | Cast    | 24,000                 | 5                       | 29,000                                               |
| 7569     | Wrought | 38,000                 | 6                       | 43,000                                               |
| 7570     | do      | 43,000                 | 3                       | 54,000                                               |
| 7573     | do      | 42,000                 | 3                       | 50,000                                               |
| VM546    | do      | 50,000                 | 6                       | 57,000                                               |

40 The tensile and creep strengths of these precipitation hardened steels exceed those of the high strength stainless steels discussed previously. Although a hot worked or as welded alloy will age harden in service at temperatures above about 1100° F., it is preferred to solution treat the alloy for about 1 hour in the temperature range of 1700 to 2100° F. and age to a hardness exceeding 250 diamond pyramid hardness at room temperature by holding for about 16 to 100 hours in the temperature range of about 1150° F. to 1350° F. Aluminum up to about 0.3% may be substituted for part of the titanium in these alloys.

45 The precipitation hardenable weldable stainless steels of this invention comprise by weight from 14% to 18% chromium, from 15% to 30% nickel, from 9% to 14% manganese, from 1% to 3% molybdenum, the manganese plus molybdenum being from 11% to 16% total, up to 0.5% vanadium, up to 0.015% boron, up to 0.03% zirconium, 0.01% to 0.06% carbon, 0.01% to 0.06% nitrogen, up to 0.4% silicon, up to 0.3% aluminum, from 1.5% to 2.5% titanium and the balance iron and incidental impurities.

50

Table XXVI

## COMPOSITIONS OF PRECIPITATION HARDENABLE, WELDABLE STAINLESS STEELS IN WEIGHT PERCENT (BALANCE IRON PLUS IMPURITIES)

| Heat No. | Cr    | Ni | Mn   | Si    | Mo   | V   | C    | N     | B     | Zr   | Ti   |
|----------|-------|----|------|-------|------|-----|------|-------|-------|------|------|
| 7569     | 16    | 25 | 11.4 | .15   | 1.02 | .27 | .037 | .009  | .0037 | .027 | 1.34 |
| 7570     | 16    | 25 | 9.74 | .15   | 1.47 | .27 | .032 | .0088 | .017  | .017 | 1.58 |
| 7573     | 14.25 | 25 | 11   | .12   | 2.25 | .25 | .03  | .05   | .005  | .015 | 1.9  |
| VM546    | 14    | 25 | 11.5 | ----- | 2    | .25 | .01  | ----- | .005  | .01  | 1.8  |

The preferred range of the precipitation hardenable weldable stainless steels comprises from 14% to 18% chromium, from 18.5% to 26% nickel, from 11% to 13% manganese, from 1% to 3% molybdenum, with the manganese plus molybdenum being from 12% to 15% total, from 0.15% to 0.35% vanadium, from 0.002% to 0.015% boron, from 0.002% to 0.03% zirconium, from 0.01% to 0.04% carbon, from 0.01% to 0.04% nitrogen, up to 0.25% silicon, up to 0.3% aluminum, from 1.75% to 2.25% titanium, and balance iron and incidental impurities. In both the broad and narrower ranges of these alloys the  $F(c)$  value is greater than 14 and the  $\phi(c)$  value is from 1 to 3.75.

To illustrate the resistance of the precipitation hardenable stainless steel to hot-cracking,  $\frac{5}{32}$  diameter rods of heat VM546 were TIG welded in a U groove  $1\frac{1}{16}$ " deep in a  $1\frac{1}{8}$ " thick plate of heat XMM 2284. No fissures were found in side bends of this fully austenitic weld.

The previously described modifications of my basic wrought or cast base metals may be joined together or to other commercial stainless steel base metals by resistance welding, by tungsten inert gas welding, by fusion welding with electrodes and wire having compositions within the scope of this invention or with commercially available crack-resistant electrodes and wire, using various existing processes. In addition, it has been found advantageous on occasion to use the crack-resistant welding electrodes of this invention to weld commercial stainless steels and other special stainless steels and alloys.

and other special stainless steels and alloys.

While the discussion of welding electrodes herein has been directed primarily to alloy compositions from which electrodes may be made, and which electrodes include substantially all the alloying elements in the desired proportions for the deposited alloy, additional amounts of the alloying elements may be included in the electrode coating in quantity sufficient to compensate for losses which occur in the welding process so as to produce the desired alloy in the weld bead. Even very substantial amounts of one or more alloying components, such as manganese, may be added through the flux coating on electrodes which may otherwise be deficient in these components.

It should be understood that the good tensile and creep properties of the alloys of this invention have not been achieved at the expense of the weldability and castability of the alloys, but instead, by the unique combination of alloying ingredients specified for my stainless steels, alloys having greatly reduced susceptibility to various forms of hot-cracking have been produced. By contrast, many of the standard stainless steels have a marginal resistance to cracking, and for many applications they are unreliable when welded or cast.

While the above description sets forth certain beliefs and theories of how the components of the various alloy compositions mentioned in the preceding discussions may be selected and proportioned and an explanation of how certain results are obtained, it should be understood that these beliefs, theories and explanations are not controlling inasmuch as there may be other factors involved, since regardless thereof, the alloys disclosed herein possess the novel properties given independent of the explanation set forth.

Although the present invention has been described with particular reference to preferred embodiments, it will be apparent to those skilled in the art that variations and modifications may be made without departing from the essential spirit and scope of the invention. It is intended to include all such variations and modifications.

I claim as my invention:

1. An austenitic stainless steel alloy of good weldability comprising, by weight, from 14% to 20% chromium, from 15% to 30% nickel, from 7.5% to 15% manganese, from 0.5% to 3.75% molybdenum, the total of manganese and molybdenum lying in the range from 9% to 16%, from 0.01% to 0.08% carbon, from 0.01%

to 0.35% nitrogen, up to about 1% silicon, up to 1% vanadium, up to 0.03% boron, up to 0.06% zirconium, up to 1.5% columbium, up to 2.5% titanium and the balance iron and small amounts of incidental impurities, the  $\phi(c)$  value of the alloy being greater than 1 to insure an adequate level of strength and rupture ductility and being less than 3.75 to insure that serious loss of impact strength after long time service at elevated temperatures does not occur, the  $F(c)$  value of the alloy being greater than 14 to assure that the alloy is fully austenitic.

10 to assure that the alloy is fully austenitic.  
15 2. An austenitic stainless steel alloy of good weldability comprising, by weight, from 14% to 20% chromium, from 15% to 30% nickel, from 7.5% to 15% manganese, from 0.5% to 3.75% molybdenum, the total of manganese and molybdenum lying in the range from 9% to 16%, from 0.01% to 0.08% carbon, from 0.01% to 0.35% nitrogen, up to about 1% silicon, at least one element selected from the group consisting of vanadium, boron and zirconium, vanadium when present amounting to from 0.15% to 0.5%, boron when present amounting to from 0.002% to 0.03%, zirconium when present amounting to from 0.002% to 0.06%, and the balance iron and small amounts of incidental impurities, the  $\phi(c)$  value of the alloy lying in the range from 1 to 3.75 and the  $F(c)$  value of the alloy being greater than 14, the alloy being  
20 resistant to hot-tearing and hot-cracking.  
25

3. A weldable fully austenitic stainless steel alloy consisting essentially of, by weight, from 14% to 18% chromium, from 15% to 6% nickel, from 9% to 14% manganese, from 1% to 3% molybdenum, the total of manganese and molybdenum lying in the range from 12% to 15%, from 0.01% to 0.06% carbon, from 0.01% to 0.25% nitrogen, up to about 0.6% silicon, up to 1% vanadium, up to 0.02% boron, up to 0.04% zirconium, and the balance iron and small amounts of incidental impurities, the  $\phi(c)$  value of the alloy lying in the range from 1 to 3.75 and the  $F(c)$  value of the alloy being greater than 14, the alloy characterized by good resistance to hot-tearing and hot-cracking and therefore being especially suitable for massive castings and for wrought members of welded unitary structures and for welding rod and electrodes.

4. A fully austenitic stainless steel alloy having excellent weldability and being especially suited for vessels, conduits and allied structures which are to be used at cryogenic temperatures, the alloy consisting essentially of, by weight, from 14% to 18% chromium, from 18.5% to 22% nickel, from 8% to 13% manganese, from 1% to 3% molybdenum, the total of manganese and molybdenum lying in the range from 11% to 16%, from 0.01% to 0.06% carbon, from 0.01% to 0.25% nitrogen, from 0.08% to 1% silicon, and the balance iron except for small amounts of impurities, the  $F(c)$  value of the alloy being greater than 14, and the austenitic structure of the alloy being stable even under deformation at the temperature of liquid helium.

5. The alloy of claim 4 containing from 0.25 to 1.5% of a stabilizing element selected from the group consisting of titanium and columbium.

60 6. A principally austenitic, highly weldable crack resistant stainless steel alloy, particularly suitable for castings and for welding electrodes, in which improved resistance to hot-cracking and hot-tearing is provided by the presence of from 2% to 10% delta ferrite therein, the alloy consisting essentially of, by weight, from 14% to 18% chromium, from 5% to 15% nickel, from 8% to 13% manganese from 1% to 3% molybdenum the total of manganese and molybdenum lying in the range from 11% to 16%, from 0.01% to 0.08% carbon, from 0.01% to 0.09% nitrogen, from 0.08% to 1% silicon and the balance iron except for small amounts of incidental impurities, the  $\phi(c)$  value of the alloy lying in the range from 1 to 3.75 and the F(c) value of the alloy being from 7.5 to 11.5.

6 75 7. An austenitic stainless steel alloy having relatively

high strength and good weldability consisting essentially of, by weight, from 14% to 18% chromium, from 18.5% to 22% nickel, from 8% to 13% manganese, from 1% to 3% molybdenum, the total of manganese and molybdenum lying in the range from 11% to 16%, from 0.01% to 0.06% carbon, from 0.10% to 0.35% nitrogen, at least one element selected from the group consisting of vanadium, boron and zirconium, vanadium when present amounting to from 0.15 to 0.5%, boron when present amounting to from 0.002% to 0.03%, zirconium when present amounting to from 0.002% to 0.06%, up to 0.6% silicon, and the balance iron and small amounts of incidental impurities, the  $\phi(c)$  value of the alloy lying in the range from 1 to 3.75 and the  $F(c)$  value of the alloy being greater than 14.

8. The alloy of claim 7 containing from 0.25% to 1.5% of a stabilizing element selected from the group consisting of titanium and columbium.

9. An austenitic stainless steel alloy having good weldability in which the alloy constituents are balanced to yield a high level of strength without forming undue amounts of the embrittling sigma phase, the alloy consisting essentially of, by weight, from 14% to 16% chromium, from 20% to 24% nickel, from 8% to 13% manganese, from 1.5% to 3% molybdenum, the total of manganese and molybdenum being from 11% to 16%, from 0.02% to 0.06% carbon, from 0.1% to 0.25% nitrogen, up to 0.4% silicon, from 0.15% to 0.35% vanadium, from 0.003% to 0.02% boron, from 0.003% to 0.04% zirconium, and the balance iron and small amounts of impurities, the  $\phi(c)$  value of the alloy lying in the range from 1 to 3.75 and the  $F(c)$  value of the alloy being greater than 14.

10. A precipitation hardenable austenitic stainless steel alloy having high strength when aged and substantial weldability, consisting essentially of, by weight, from 14% to

18% chromium, from 15% to 30% nickel, from 9% to 14% manganese, from 1% to 3% molybdenum, the total of manganese and molybdenum lying in the range from 11% to 16%, from 0.01% to 0.06% carbon, up to 0.4% silicon, from 0.01% to 0.06% nitrogen, up to 0.5% vanadium, up to 0.015% boron, up to 0.03% zirconium, up to 0.03% zirconium, up to 0.3% aluminum, from 1.5% to 2.5% titanium to provide the precipitation hardening characteristic, and the balance iron except for small amounts of incidental impurities, the  $\phi(c)$  value of the alloy lying in the range from 1 to 3.75 and the  $F(c)$  value being greater than 14.

11. An austenitic stainless steel alloy of good weldability comprising, by weight, from 14% to 20% chromium, from 15% to 30% nickel, from 7.5 to 15% manganese, from 0.5% to 3.75% molybdenum, the total of manganese and molybdenum lying in the range from 9% to 16%, from 0.01% to 0.08% carbon, from 0.01% to 0.35% nitrogen, up to about 1% silicon, from 0.15% to 0.35% vanadium, from 0.003% to 0.02% boron, from 0.003% to 0.04% zirconium, and the balance iron and small amounts of incidental impurities, the  $\phi(c)$  value of the alloy lying in the range from 1 to 3.75 and the  $F(c)$  value of the alloy being greater than 14, the alloy being resistant to hot tearing and hot-cracking.

#### References Cited by the Examiner

##### UNITED STATES PATENTS

30 2,894,833 7/59 Linnert et al. ----- 75—128  
35 2,955,034 10/60 Korchynsky ----- 75—128

##### FOREIGN PATENTS

476,413 12/37 Great Britain.

35 DAVID L. RECK, Primary Examiner.